



US008403146B2

(12) **United States Patent**  
**Hurd et al.**

(10) **Patent No.:** **US 8,403,146 B2**  
(45) **Date of Patent:** **Mar. 26, 2013**

(54) **COLLECTORS**

(75) Inventors: **Phillip W. Hurd**, Conyers, GA (US);  
**John B. Hines**, Atlanta, GA (US)

(73) Assignee: **Georgia-Pacific Chemicals LLC**,  
Atlanta, GA (US)

(\*) Notice: Subject to any disclaimer, the term of this  
patent is extended or adjusted under 35  
U.S.C. 154(b) by 435 days.

(21) Appl. No.: **12/496,122**

(22) Filed: **Jul. 1, 2009**

(65) **Prior Publication Data**

US 2010/0000913 A1 Jan. 7, 2010

**Related U.S. Application Data**

(60) Provisional application No. 61/077,725, filed on Jul. 2,  
2008.

(51) **Int. Cl.**

**B03D 1/008** (2006.01)  
**B03D 1/02** (2006.01)

(52) **U.S. Cl.** ..... **209/166**

(58) **Field of Classification Search** ..... 209/166,  
209/167

See application file for complete search history.

(56) **References Cited**

U.S. PATENT DOCUMENTS

2,395,639 A 2/1946 Monson et al.  
2,652,150 A \* 9/1953 Weinig ..... 209/166  
3,275,141 A \* 9/1966 Adams et al. ..... 209/166  
4,301,003 A \* 11/1981 Hsieh ..... 209/166  
4,585,550 A \* 4/1986 Avotins et al. ..... 209/166  
4,589,980 A \* 5/1986 Keys ..... 209/166  
4,927,669 A 5/1990 Knox et al.  
8,133,970 B2 \* 3/2012 Hurd et al. ..... 530/211  
2006/0151360 A1 7/2006 Wright et al.  
2006/0151397 A1 7/2006 Wright et al.  
2007/0000839 A1 1/2007 Wright et al.  
2007/0012630 A1 1/2007 Wright et al.  
2008/0017552 A1 1/2008 Wright et al.  
2008/0029460 A1 2/2008 Wright et al.

FOREIGN PATENT DOCUMENTS

CN 1073895 A 7/1993  
CN 1343531 A 4/2002

GB 584305 A 1/1947  
GB 2163975 A \* 3/1986  
SU 666709 A 5/1982  
WO 91/16986 A1 11/1991

OTHER PUBLICATIONS

Georgia-Pacific Chemicals LLC, Material Safety Data Sheet for  
XTOL® 0530 Rosin Fortified Distilled Tall Oil, effective date Oct.  
30, 1997, six pages.

Georgia-Pacific Chemicals LLC, Material Safety Data Sheet for  
LYTOR® 100 Tall Oil Resin, effective date Jan. 22, 2001, seven  
pages.

Georgia-Pacific Chemicals LLC, Material Safety Data Sheet for  
XTOL® 0520 Distilled Tall Oil, effective date Dec. 9, 2004, seven  
pages.

Georgia-Pacific Chemicals LLC, Material Safety Data Sheet for  
XTOL® MTO Modified Tall Oil, effective date May 23, 2007, seven  
pages.

Georgia-Pacific Chemicals LLC, Material Safety Data Sheet for  
XTOL® 0542 Rosin Fortified Distilled Tall Oil, effective date Oct. 9,  
2007, seven pages.

Georgia-Pacific Chemicals LLC, Material Safety Data Sheet for  
XTOL® 692 Modified Tall Oil, effective date Oct. 30, 2007, seven  
pages.

Georgia-Pacific Chemicals LLC, Material Safety Data Sheet for  
XTOL® 690 Modified Tall Oil, effective date Jan. 23, 2008, seven  
pages.

Georgia-Pacific Chemicals LLC, Material Safety Data Sheet for  
XTOL® 304 Tall Oil Fatty Acids, effective date Apr. 4, 2008, six  
pages.

Georgia-Pacific Chemicals LLC, Material Safety Data Sheet for  
XTOL® 100 Tall Oil Fatty Acids, effective date Apr. 14, 2008, six  
pages.

Georgia-Pacific Chemicals LLC, Material Safety Data Sheet for  
XTOL® 101 Tall Oil Fatty Acids, effective date Apr. 14, 2008, six  
pages.

Georgia-Pacific Chemicals LLC, Material Safety Data Sheet for  
XTOL® 300 Tall Oil Fatty Acids, effective date Apr. 14, 2008, six  
pages.

International Search Report and Written Opinion of the International  
Search Authority mailed Jan. 22, 2010.

\* cited by examiner

*Primary Examiner* — Thomas M Lithgow

(74) *Attorney, Agent, or Firm* — Ram W. Sabinis

(57) **ABSTRACT**

Collectors for froth flotation including oxidized fatty acid  
compositions and oxidized and maleated compositions. In  
particular, use of oxidized tall oil compositions and oxidized  
and maleated fatty acid compositions are disclosed.

**24 Claims, 5 Drawing Sheets**



FIG. 1



FIG. 2



FIG. 3



FIG. 4



FIG. 5

## 1 COLLECTORS

### CROSS-REFERENCE TO RELATED APPLICATION

This application claims priority to U.S. Provisional Patent Application No. 61/077,725 filed Jul. 2, 2008, the disclosure of which is incorporated herein in its entirety by this reference.

### TECHNICAL FIELD

This disclosure relates to processing of ore into minerals and gangue. This disclosure also relates to collectors used in froth flotation, and methods of using the collectors in froth flotation.

### BACKGROUND

Froth flotation is used for beneficiating ores. In particular, froth flotation can be used for separating valuable minerals in an ore from their associated gangue, or for separating the valuable minerals from one another. Froth flotation involves mixing an aqueous slurry containing finely ground ore particles with a frothing or foaming agent to produce a froth. Ideally, ore particles that contain the desired mineral are preferentially attracted to the froth because of an affinity between the froth and the exposed mineral on the surfaces of the ore particles. The resulting beneficiated minerals are then collected by separating them from the froth.

The ability of a mineral to float is related to its surface properties. Chemical reagents known as "collectors" are used to modify surface properties of minerals, and may be added to the slurry to increase the selectivity and efficiency of the separation process.

Because of the large scale on which mining operations are typically conducted and the large difference in value between the desired mineral and the associated gangue, even relatively small increases in separation efficiency provide substantial gains in productivity.

### SUMMARY

This disclosure provides collectors for use in froth flotation, and methods of using the collectors in froth flotation. In some embodiments, the collector comprises an oxidized fatty acid composition. In some embodiments, the collector comprises an oxmal composition, as defined below.

In some embodiments, the method for froth flotation comprises floating a mineral using a collector comprising one or more of an oxidized clean fatty acid composition, an oxmal composition, and mixtures thereof. In some embodiments, the collector can be an oxidized fatty acid composition, such as an oxidized tall oil fatty acid composition. In some embodiments, the collector can be an oxmal composition.

In some embodiments, the method of froth flotation (e.g., phosphate froth flotation) comprises the use of a collector made by the process of: a) providing a clean fatty acid composition; and b) oxidizing the clean fatty acid composition; to separate a mineral from gangue. In some embodiments, the collector can be made by the process of: a) providing a fatty acid composition; b) maleating the fatty acid composition; and c) oxidizing the fatty acid composition.

In some embodiments, the froth flotation process comprises collecting a mineral using an oxidized fatty acid composition, wherein the oxidized fatty acid composition can have one or more of: (1) less than 2.5% by weight of a

## 2

plant-derived amine; (2) at least 65% by weight of an oxidized fatty acid; (3) less than 5% by weight of a tall oil pitch; or (4) less than 20% by weight of a fuel oil or furnace oil.

In some embodiments, a froth flotation process is provided, 5 the method comprising collecting a mineral using an oxidized fatty acid composition, wherein the oxidized fatty acid composition has an acid value of at least about 80. In some embodiments, the acid value is at least about 110. In some embodiments, the acid value is between about 120 and 150.

10 Further provided herein are embodiments for a froth flotation process comprising collecting a mineral using an oxidized fatty acid composition or an oxmal composition and providing a yield and/or grade of the mineral which is higher than a yield and/or grade of the mineral provided by a fatty acid composition.

15 In any of the above embodiments, the collector of any of the above can be an anionic collector. The anionic collector can have a counter cation chosen from for example Li<sup>+</sup>, Na<sup>+</sup>, K<sup>+</sup>, NH4<sup>+</sup>, alkyl ammonium ions, and imidazoline cations. In any of the above embodiments, the mineral to be floated can be chosen from phosphate, barite, fluorite, feldspar, potash, fluorspar, magnesite, scheelite, celestite, anglesite, alunite, bauxite, gypsum, kainite, biotite, calcite, dolomite, albite, orthoclase, microcline, fluorspar, gypsum, anhydrite, columbite, tantalite, pyrochlore, apatite, cassiterite, wolframite, rutile, ilmenite, hematite, and kaolin. In some embodiments, the mineral is phosphate or potash.

20 In any of the above methods and embodiments, the method can further comprise the use of one or more of a frothing agent or a depressant.

25 A method of potash froth flotation is provided, the method comprising floating potash using a collector comprising an oxidized fatty acid composition or an oxmal composition.

30 Also provided herein is a method of separating a mineral from gangue, the method comprising providing an oxidized fatty acid composition or an oxmal composition to a solution of the mineral and gangue, thereby separating the mineral from the gangue.

35 40 A composition is further provided, the composition comprising a collector, wherein the collector comprises one or more of an oxidized fatty acid composition, oxmal composition, and mixtures thereof, and one or more of a frothing agent and a depressant. Also provided is a composition comprising two or more collectors, wherein at least one, but not all, of the collectors is an oxidized fatty acid.

45 50 Further provided herein is a kit comprising a collector and one or more of a frothing agent and a depressant, wherein the collector comprises one or more of an oxidized fatty acid composition, oxmal composition, and mixtures thereof.

55 In any of the previous kit embodiments, the kit can further comprises instructions for floating a mineral.

60 In any of the kit embodiments, the kit can further comprises a label that indicates that the contents are to be used in froth flotation of a mineral.

The details of one or more non-limiting embodiments of the invention are set forth in the accompanying drawings and the description below. Other embodiments of the invention should be apparent to those of ordinary skill in the art after consideration of the present disclosure.

### DESCRIPTION OF DRAWINGS

65 FIG. 1 illustrates the effects of collector type and dosage on phosphate flotation recovery.

FIG. 2 details the effects of collector type and dosage on phosphate flotation product P<sub>2</sub>O<sub>5</sub> grade.

FIG. 3 shows the effects of collector type and dosage on the soils grade of flotation product.

FIG. 4 illustrates the effects of collector type and dosage on phosphate separation efficiency.

FIG. 5 details P<sub>2</sub>O<sub>5</sub> recovery vs. A.I. rejection.

## DETAILED DESCRIPTION

### I. Definitions

Unless defined otherwise, all technical and scientific terms used herein have the same meaning as is commonly understood by one of ordinary skill in the art to which this disclosure belongs. All patents, applications, published applications, and other publications are incorporated by reference in their entirety. In the event that there is a plurality of definitions for a term herein, those in this section prevail unless stated otherwise.

An “oxidized fatty acid” is a compound, or salt thereof, comprising at least two or more fatty acid backbone structures, wherein each backbone structure is linked to one other backbone structure by a bridging group chosen from a direct bond, an ether linkage, or a peroxide linkage located at a non-terminal position of each backbone structure, or is a fatty acid that has been oxidized by any means known in the art.

An “oxidized fatty acid composition” is a composition comprising an oxidized fatty acid, a mixture of two or more oxidized fatty acids, or an oil that has been oxidized by any means known in the art. Non-limiting examples of oxidized fatty acid compositions include tall oils, which have been oxidized; animal oils, which have been oxidized; plant oils, which have been oxidized; algal derived oils, which have been oxidized; and microbially derived oils, which have been oxidized. In some embodiments, oxidized fatty acid compositions can also include one or more non-reacted or partially reacted species, such as non-oxidized fatty acids, rosin acids, and mixtures thereof.

A “clean fatty acid composition” is a composition comprising one or more fatty acids, wherein the composition does not contain one or more of tall oil pitch; an amine (e.g., an amine derived from a plant); and sarcosine. In some embodiments, a clean fatty acid composition also does not contain fuel oil and/or furnace oil.

An “oxidized clean fatty acid composition” is a composition comprising an oxidized fatty acid, a mixture of two or more oxidized fatty acids, or an oil that have been oxidized by any means known in the art, wherein the oxidized clean fatty acid composition does not contain one or more of tall oil pitch; an amine (e.g., a biogenic amine, such as an amine derived from a plant, or a synthetic amine); or sarcosine. In some embodiments, an oxidized clean fatty acid composition also does not contain fuel oil and/or furnace oil. Non-limiting examples of oxidized clean fatty acid compositions include tall oils, which have been oxidized; animal oils, which have been oxidized; plant oils, which have been oxidized; algal derived oils, which have been oxidized; and microbially derived oils, which have been oxidized. In some embodiments, oxidized clean fatty acid compositions can also include one or more non-reacted or partially reacted species, such as non-oxidized clean fatty acids, rosin acids, and mixtures thereof.

An “oxidized and maleated compound” (hereinafter an “oxmal compound”) is a compound, or salt thereof, comprising at least two or more hydrocarbon-based backbone structures, wherein at least one of the backbone structures is substituted by at least one of an  $\alpha,\beta$  unsaturated carboxylic acid or anhydride, and further wherein each backbone structure is linked to one other backbone structure by a bridging group

chosen from a direct bond, an ether linkage, or a peroxide linkage located at a non-terminal position of each backbone structure. In some embodiments, the hydrocarbon-based backbone structure is a C<sub>10</sub>-C<sub>24</sub> hydrocarbon. In some 5 embodiments, the hydrocarbon-based backbone is a C<sub>10</sub>-C<sub>24</sub> fatty acid or rosin acid. In some embodiments, the  $\alpha,\beta$  unsaturated carboxylic acid or anhydride is maleic anhydride, fumaric acid, acrylic acid, or methacrylic acid (herein acrylic acid and methacrylic acid are generally referred to in the aggregate or alternative as (meth)acrylic acid). In some 10 embodiments, the  $\alpha,\beta$  unsaturated carboxylic acid or anhydride is a biogenically derived unsaturated carboxylic acid or anhydride. Non-limiting examples of oxmal compounds include dimers and trimers of fatty acids, rosin acids and 15 mixtures thereof, linked at an intermediary position along the fatty acid or rosin acid backbone by a direct bond, an ether linkage, or a peroxide linkage, and wherein each of the fatty acids and rosin acids is substituted by a maleic anhydride, fumaric acid, or (meth)acrylic acid.

An “oxidized and maleated composition” (hereinafter an “oxmal composition”) is a composition comprising one or more oxmal compounds, wherein when the composition comprises more than one oxmal compound, the oxmal compounds can be the same or different. Non-limiting examples 20 of oxmal compositions include tall oils, which have been maleated and oxidized; animal oils, which have been maleated and oxidized; plant oils, which have been maleated and oxidized; algal derived oils, which have been maleated and oxidized; and microbially derived oils, which have been maleated and oxidized. In some embodiments, oxmal compositions 25 can also include one or more non-reacted or partially reacted species, such as non-maleated dimers, trimers, etc of fatty acids, rosin acids, and mixtures thereof.

The phrase “a compound, which has been maleated and 30 oxidized” is used interchangeably with “a maleated and oxidized compound”. The phrase “a composition, which has been maleated and oxidized” is used interchangeably with “a maleated and oxidized composition.” The phrase “oxidized and maleated” is used interchangeably with “maleated and 35 oxidized.”

Wherever the phrase “for example”, “such as”, and the like 40 are used herein, the phrase “and without limitation” is understood to follow unless explicitly stated otherwise. Therefore, “for example tall oil” means “for example and without limitation tall oil”. Similarly all examples herein are non-limiting unless explicitly stated otherwise.

As used herein, the terms “maleated,” “maleation,” and the 45 like refer to the modification of hydrocarbon-based backbone structures having one or more sites of unsaturation (e.g., C<sub>18</sub>-fatty acids, such as linoleic acid and oleic acid), which introduces additional carboxylic moieties onto the molecules by reaction with one or more  $\alpha,\beta$  unsaturated carboxylic acids or anhydrides. In some embodiments, an  $\alpha,\beta$  unsaturated carboxylic acid or anhydride is chosen from maleic anhydride, fumaric acid, acrylic acid, and methacrylic acid (herein 55 acrylic acid and methacrylic acid are generally referred to in the aggregate or alternative as (meth)acrylic acid). In some embodiments, an  $\alpha,\beta$  unsaturated carboxylic acid or anhydride is a biogenically derived unsaturated carboxylic acid or anhydride.

As used herein, “acid functionality” in addition to its 60 traditional meaning, also encompasses groups which are hydrolyzable such as anhydride groups.

As used herein, the terms “carboxylic moiety” and “carboxylic moieties” are also intended to include the anhydride structure formed by the condensation reaction between two carboxyl groups.

As used herein, "tall oil fatty acid" or "TOFA", consistent with industry standards, encompasses compositions which include not only fatty acids, but also rosin acids and/or unsaponifiables. TOFAs are generally produced as a distillation fraction of crude tall oil and therefore contain saturated and unsaturated fatty acids, rosin acids, and mixtures thereof.

The term "mineral" is used to encompass a pure mineral as well as ore which has been beneficiated.

As used herein, "alkyl," "alkenyl" and "alkynyl" carbon chains, if not specified, should be broadly interpreted, for example to encompass substituted or unsubstituted, straight, branched, and cyclic "chains."

As used herein, "polyolefin oligomers" in addition to its traditional meaning, also encompasses oligomers having one site of unsaturation.

As used herein, "about" is meant to account for variations due to experimental error.

## II. Methods of Froth Flotation

Provided herein are methods of froth flotation comprising floating a mineral using compounds and compositions, described herein, as froth flotation collectors. In some embodiments, the method comprises floating a mineral using an oxidized fatty acid as a collector in a froth flotation process. In some embodiments, the method comprises floating a mineral using an oxidized fatty acid composition as a collector in a froth flotation process. In some embodiments, the method comprises floating a mineral using an oxidized clean fatty acid composition as a collector in a froth flotation process. In some embodiments, the method comprises floating a mineral using an oxmal compound as a collector in a froth flotation process. In some embodiments, the process comprises floating a mineral using an oxmal composition as a collector in a froth flotation process.

In some embodiments, the method comprises floating a mineral using at least one collector chosen from oxidized fatty acids, oxidized fatty acid compositions, oxidized clean fatty acid compositions; oxmal compounds, oxmal compositions, and mixtures thereof.

In accordance with the invention, collectors as described herein can be used in similar froth flotation applications as fatty acid collectors. For example, the collectors described herein can be used to float phosphate, barite, fluorite, feldspar, potash, fluorspar, magnesite, scheelite, celestite, anglesite, alumite, bauxite, gypsum, kainite, biotite, calcite, dolomite, albite, orthoclase, microcline, fluorspar, gypsum, anhydrite, columbite, tantalite, pyrochlore, apatite, cassiterite, wolframite, rutile, ilmenite, hematite, and kaolin. In some embodiments, the mineral is phosphate or potash. In some embodiments, the mineral is phosphate. In some embodiments, the mineral is potash.

In some embodiments, certain of the collectors, as described herein, exhibit improved performance when compared to fatty acid collectors currently in use. For example, in some embodiments, certain of the collectors exhibit increased yield of a mineral when compared to the fatty acid collectors (e.g., fatty acids derived from tall oil, plant oil, animal oil, or mixtures thereof) currently in use. In some embodiments, certain of the collectors described herein exhibit improved grade of a mineral when compared to the fatty acid collectors currently in use. In some embodiments, less collector is required to float a mineral compared to the fatty acid collectors currently in use.

See, for example, Example 1 which illustrates the ability of an oxidized tall oil fatty acid and an oxmal composition, each in accordance with a certain embodiment of the invention, to increase various aspects of phosphate collection, including percent phosphate flotation recovery,  $P_2O_5$  product grade,

sols product grade, phosphate separation efficiency, and  $P_2O_5$  recovery vs. A.I. rejection when compared to various experimental collectors. In all conditions studied the oxidized fatty acid out performed all other collectors evaluated, including two commercial phosphate collectors. The oxmal composition was found to be superior to a tall oil fatty acid composition (XTOL® 100) which is commonly used as a component of a commercial phosphate collector.

A collector, as described herein, can be used in combination with other compounds, for example, frothing agents, depressants, additional collectors, activators, and modifiers. In some embodiments, a collector, as described herein, can comprise at least about 65% by weight (e.g., at least about 70% by weight, at least about 75% by weight, at least about 80% by weight, at least about 82% by weight, at least about 85% by weight, at least about 94% by weight, at least about 95% by weight, at least about 97% by weight, at least about 98% by weight, at least about 99% by weight, and at least about 99.5% by weight) of a collector composition. In some embodiments, the collector is an oxidized fatty acid compound. In some embodiments, the collector is an oxidized fatty acid composition. In some embodiments, the collector is an oxmal compound. In some embodiments, the collector is an oxmal composition.

A frothing agent can be used to lower the interfacial tension of the aqueous slurry with air and control the size of the air bubbles. These properties can increase the strength and stability of the surface froth, thus improving the ability of the surface froth to support the mineral particles that float until they are removed from the system. Non-limiting examples of frothing agents include pine oil, methyl isobutyl carbitol (MIBC) and other alcohols of similar molecular weight, glycols and polyglycols, glycol and polyglycol ethers of aliphatic alcohols such as cyclohexanol. In some embodiments, a collector is combined with a frothing agent prior to addition to a flotation cell. In some embodiments, a collector and a frothing agent are added individually. In some embodiments, a collector is added to a flotation cell prior to addition of a frothing agent. In some embodiments, a collector is added to a flotation cell following addition of a frothing agent.

A depressant can decrease or prevent the entry of undesired minerals into the froth by precipitating deleterious ions that could interfere with collection or by coating selected minerals to decrease or prevent collector attachment. Non-limiting examples of depressants include urea formaldehyde polymers and oligomers, see, for example, U.S. Patent Publication Nos. 2008/0029460; 2008/0017552; 2007/0012630; 2007/0000839; 2006/0151397; and 2006/0151360. Further examples of depressants include: cyanide salts; sodium sulfide/hydrosulphide; sulphites; waterglass; polysaccharides such as starch, chemically modified polysaccharides like carboxymethylcellulose (CMC); natural gums like guar gum, agar, alginic acid, glucan, carrageenan, chicle gum, gellan gum, glucomannan, gum arabic, locust bean gum, psyllium seed husks, alginates, spruce gum, tara gum, and xanthan gum; and chemically modified natural gums. In some embodiments, a collector is combined with a depressant prior to addition to a flotation cell. In some embodiments, a collector and a depressant are added individually. In some embodiments, a collector is added to a flotation cell prior to addition of a depressant. In some embodiments, a collector is added to a flotation cell following addition of a depressant.

Depending on the ore to be beneficiated and its condition, it can sometimes be desirable to use more than one collector in a froth flotation process. In some embodiments, a collector, as described herein, can be used in combination with one or more additional collectors. Additional collectors can be cho-

sen from, for example, ionic and nonionic collectors. Ionic collectors can be chosen from an anionic collector (e.g., xanthates, thiophosphates, organic sulfides, carboxylic collectors, and sulfoxy collectors), a cationic collector (e.g., amines and amine salts), and an amphoteric collector. Nonionic collectors can include nonpolar and heteropolar collectors. In some embodiments, an additional collector is chosen from amines, fatty acids, fuel oil, kerosene, petroleum sulfonate (e.g., lignin), thionocarbamates (e.g., ethyl isopropyl thionocarbamate and methyl butyl thionocarbamates), xanthates (e.g., isopropyl xanthate, amyl xanthate, butyl xanthate, and ethyl xanthate), tall oil, thiophosphates (e.g., dicesyl thiophosphate, di-sec-butyl thiophosphate, diamyl thiophosphate, and diethyl thiophosphate), oleic acid, xanthogen formate, sodium dodecyl sulfate, and mercaptans (e.g., dodecyl mercaptan). In some embodiments, a collector, as described herein, is combined with at least one additional collector. In some embodiments, a collector is combined with at least two additional collectors. In some embodiments, the combination of collectors are combined prior to addition to a flotation cell. In some embodiments, each collector is added individually to a flotation cell.

Activators can be used to promote coating of the collector onto the desired mineral. In some embodiments, an activator can be an inorganic commodity chemical, such as copper ions (e.g., sulfates and chloride), aluminum salts (e.g., nitrates and sulfates), sodium sulfide, silicates (e.g., sodium and potassium), carbonates (e.g., sodium), hydroxides (e.g., sodium and calcium), lead acetate, and sodium hydrosulfide. In some embodiments, an activator can reduce the amount of collector added to a flotation cell. In some embodiments, an activator can reduce collector consumption. In some embodiments, an activator can increase the preference of a collector for a particular mineral.

A modifier can be used to increase selectivity of a collector. Non-limiting examples of modifiers include: lime, soda ash, alum, ammonia, caustic soda, phosphates, sodium silicate, sulfur dioxide, lignosulfonate, cationic modifiers (e.g.,  $\text{Ba}^{2+}$ ,  $\text{Ca}^{2+}$ ,  $\text{Cu}^+$ ,  $\text{Pb}^{2+}$ ,  $\text{Zn}^{2+}$ , and  $\text{Ag}^+$ ), anionic modifiers (e.g.,  $\text{SiO}_3^{2-}$ ,  $\text{PO}_4^{3-}$ ,  $\text{CN}^-$ ,  $\text{CO}_3^{2-}$ , and  $\text{S}^{2-}$ ), organic modifiers (e.g., Dextrin, starch, glue, and carboxymethylcellulose), sulfuric acid, and hydrochloric acid. In some embodiments, a modifier can alter the pH of an aqueous slurry. In some embodiments, a modifier can increase the pH of an aqueous slurry. For example, the pH of an aqueous slurry can be increased to a pH ranging from about 9 to about 12. In some embodiments, a modifier can decrease the pH of an aqueous slurry. For example, the pH of an aqueous slurry can be decreased to a pH ranging from about 2 to about 3. In some embodiments, a collector and a modifier are used in combination. In some embodiments, a collector and a modifier are used individually.

In some embodiments, a collector as described herein (e.g., an oxidized fatty acid composition) can be combined with other minor components.

In some embodiments, a collector composition can include less than about 2.5% by weight (e.g., less than about 2% by weight, less than about 1.75% by weight, less than about 1.5% by weight, less than about 1.25% by weight, less than about 1% by weight, less than about 0.75% by weight, less than about 0.5% by weight, less than about 0.25% by weight, less than about 0.1% by weight, and less than about 0.05% by weight) of an amine (e.g., a plant-derived amine).

In some embodiments, a collector composition can include less than about 5% by weight (e.g., less than about 4.5% by weight, less than about 4% by weight, less than about 3% by weight, less than about 2.5% by weight, less than about 2% by

weight, less than about 1.75% by weight, less than about 1.5% by weight, less than about 1.35% by weight, less than about 1.25% by weight, less than about 1% by weight, less than about 0.5% by weight, less than about 0.25% by weight, and less than about 1% by weight) of a tall oil pitch.

In some embodiments, a collector composition can include less than about 20% by weight (e.g., less than about 18% by weight, less than about 15% by weight, less than about 12% by weight, less than about 10% by weight, less than about 8% by weight, less than about 6% by weight, less than about 5% by weight, less than about 3% by weight, less than about 2% by weight, less than about 1% by weight, and less than about 0.5% by weight) of a fuel oil (e.g., diesel fuel) or furnace oil.

In some embodiments, a collector may be in a salt form. In some embodiments, a collector is in an anionic form. Any suitable counter cation may be used with an anionic collector, such as  $\text{Li}^+$ ,  $\text{K}^+$ ,  $\text{Na}^+$ ,  $\text{NH}_4^+$ , alkyl ammonium ions, and imidazoline cations. In some embodiments, a counter cation can be a divalent or trivalent cation, for example  $\text{Mg}^{2+}$ ,  $\text{Ca}^{2+}$ ,  $\text{Ba}^{2+}$ , and  $\text{Al}^{3+}$ . In some embodiments, the counter cation is  $\text{Na}^+$ . A collector salt, or soap, can be prepared, for example, by reacting the collector (e.g., an oxidized fatty acid composition, an oxidized clean fatty acid composition, or an oxmal composition) with any appropriate base (e.g.,  $\text{NaOH}$ ) to prepare the corresponding salt. See, e.g., Examples 8 and 9.

A collector, as described herein, may increase the yield of a mineral when compared to industry standard collectors (e.g., fatty acid collectors). In some embodiments, the yield is increased from about 0.5% to about 50% (e.g., 0.5%, 1%, 1.5%, 1.8%, 2%, 3%, 5%, 7.5%, 10%, 12%, 15%, 20%, 25%, 30%, 40%, and 50%). In some embodiments, the yield is increased 1.8%. In some embodiments, the yield of a mineral using a collector, as described herein, is from about 80% to about 100% (e.g., 80%, 82%, 85%, 87%, 89%, 91%, 93%, 95%, 97%, 97.5%, 98%, 98.5%, 99%, 99.2%, 99.7%, and 99.9%). In some embodiments, the yield of a mineral is 99.7%. See, e.g., Example 1.

In some embodiments, use of a collector as described herein results in improved grade mineral when compared to industry standard collectors. In some embodiments, the percent  $\text{P}_2\text{O}_5$  grade can be improved. In some embodiments, the percent sols product grade can be improved. See, e.g., Example 1.

Depending on the ore and its condition, a collector can be used in an amount ranging from about 0.04 lb per ton of ore to about 10 lb per ton or ore. In some embodiments, a collector can be used in an amount ranging from about 0.3 lb per ton of ore to about 0.9 lb per ton of ore. In some embodiments, a collector can be used in an amount of about 0.9 lb per ton of ore. See, e.g., Example 1.

Any suitable froth flotation cell and method of operation of a froth flotation cell used with fatty acids can be used with a collector as described herein. In some embodiments, the froth flotation is an anionic or positive flotation. In some embodiments, an initial anionic flotation is followed by a cationic or reverse flotation. The non-limiting examples below illustrate various embodiments of a froth flotation process (see Example 1).

In some embodiments, a froth flotation process for beneficiating an ore can include the steps of: (a) forming a slurry comprising water and particles of an ore; (b) intermixing the slurry with a collector as described herein; and (c) collecting the beneficiated ore. In some embodiments, the slurry is an aqueous slurry. In some embodiments, the froth flotation process can further include intermixing the slurry with a frothing agent. In some embodiments, the froth flotation process can further include intermixing the slurry with a depressant. In some embodiments, the frothing agent and/or the

depressant are combined with the collector prior to intermixing with the slurry. In some embodiments, the collector, frothing agent, and/or depressant are intermixed with the slurry individually.

In some embodiments, a process of separating particles of a first material from a second material in an aqueous slurry is provided. Such a process can include the steps of (a) adding a collector composition to an aqueous slurry of the materials; (b) providing air bubbles in the aqueous slurry to form bubble-particle aggregates, each of the bubble-particle aggregates having at least one of the air bubbles and at least one of the particles of the first material; and (c) allowing the bubble-particle aggregates to float in the aqueous slurry. In some embodiments, the bubble-particle aggregates further include at least one compound of a collector composition. In some embodiments, the slurry is agitated following addition of the collector composition. In some embodiments, the first material is hydrophobic and the second material is hydrophilic. In some embodiments, the collector composition increased the hydrophobicity of one of the materials.

In some embodiments, a process of floating a phosphate mineral is provided. In some embodiments, the phosphate mineral is separated from a mineral mixture. In some embodiments, the phosphate is separated from carbonate (e.g., dolomite). In some embodiments, the phosphate is separated from dolomite, calcite, quartz, and silicates. In some embodiments, the collector used is selective for phosphate. In some embodiments, an ore slurry comprising phosphate is subjected to a desliming step prior to froth flotation. In some embodiments, a collector as described herein can be used to separate phosphate from the slime fraction.

In some embodiments, a method of separating a mineral from gangues is provided, the method comprising providing an oxidized fatty acid composition to a solution of mineral and gangue, and separating the mineral from the gangue. In some embodiments, the oxidized fatty acid composition facilitates the separation of the mineral from the gangue. Without being bound by theory, in some embodiments the oxidized fatty acid composition functions as a collector. In some embodiments, a method of separating a mineral from gangues is provided, the method comprising providing an oxidized clean fatty acid composition to a solution of mineral and gangue, and separating the mineral from the gangue. In some embodiments, the oxidized clean fatty acid composition facilitates the separation of the mineral from the gangue. Without being bound by theory, in some embodiments the oxidized clean fatty acid composition functions as a collector. In some embodiments, a method of separating a mineral from gangues is provided, the method comprising providing an oxmal composition to a solution of mineral and gangue, and separating the mineral from the gangue. In some embodiments, the oxmal composition facilitates the separation of the mineral from the gangue. Without being bound by theory, in some embodiments the oxmal composition functions as a collector.

## II. Collector Compounds and Compositions

The disclosure provides oxidized fatty acid compounds, oxidized fatty acid compositions, oxidized clean fatty acid compositions, oxmal compounds, oxmal compositions, and mixtures thereof useful as collectors in froth flotation, for

example, useful for floating ore or minerals otherwise floated by fatty acids such as tall oil fatty acids or side streams of the tall oil distillation process.

### A. Oxidized Fatty Acid Compounds

Oxidized fatty acid compounds provided herein comprise at least two or more fatty acid backbone structures, wherein each backbone structure is linked to one other backbone structure by a bridging group chosen from a direct bond, an ether linkage, or a peroxide linkage located at a non-terminal position of each fatty acid backbone structure. The fatty acid backbone structure can be chosen from, for example, C<sub>10</sub>-C<sub>22</sub> fatty acids. The fatty acid backbone structure can be chosen from, for example, C<sub>16</sub>-C<sub>22</sub> fatty acids. The fatty acid backbone structure can be chosen from, for example, C<sub>16</sub>-C<sub>18</sub> fatty acids. The fatty acid backbone structure can be, for example, a C<sub>18</sub> fatty acid. The fatty acid backbone structure can be chosen from, for example, oleic, linoleic, and linolenic acid.

In some embodiments, the oxidized fatty acid compounds have two or three fatty acid backbone structures, and each of the fatty acid backbone structures is the same. For example, without limitation, each of the two or three fatty acid backbone structures can be an oleic acid. Formulas 1-4 below are examples of oxidized fatty acid compounds having backbone structures chosen from the same fatty acid. Non-limiting examples of oxidized fatty acid compounds having two fatty acid backbone structures that are the same include: oxidized decenoic acid; oxidized dodecenoic acid; oxidized cis-9-tetradecenoic acid; oxidized cis-9-hexadecenoic acid; oxidized oleic acid; oxidized linoleic acid; oxidized linolenic acid; oxidized cis-6,cis-9,cis-12,cis-15-octadecatetraenoic acid; oxidized ricinoleic acid; oxidized cis-9-eicosenoic acid; oxidized cis-11-eicosenoic acid; oxidized eicosadienoic acid; oxidized eicosatrienoic acid; oxidized arachidonic acid; oxidized eicosapentaenoic acid; oxidized erucic acid; oxidized docosadienoic acid; oxidized 4,8,12,15,19-docosapentaenoic acid; oxidized docosahexaenoic acid; and oxidized tetracosenoic acid.

In some embodiments, the oxidized fatty acid compounds have two different fatty acid backbone structures. In some embodiments, the oxidized fatty acid compounds have three different fatty acid backbone structures. For example, without limitation, one of the fatty acid backbone structures can be oleic acid and one can be linoleic acid. Formula 5 below is one example of an oxidized fatty acid compound having two different fatty acid backbone structures.

In some embodiments, an oxidized fatty acid compound may be in a salt form. For example, all or some portion of an oxidized fatty acid compound in an oxidized fatty acid composition can be in a salt form. In some embodiments, an oxidized fatty acid compound is in an anionic form. Any suitable counter cation may be used with an anionic oxidized fatty acid compound, such as Li<sup>+</sup>, K<sup>+</sup>, and Na<sup>+</sup>. In some embodiments, the counter cation is Na<sup>+</sup>. See Example 8.

Non-limiting specific structure examples of oxidized fatty acid compounds in accordance with the invention are illustrated as Formulas 1-5 below. These examples illustrate one isomeric form; other isomers (e.g., cis and trans isomers) can be prepared and accordingly are within the scope of the invention.

(I)



(II)





(III)



#### B. Oxmal Compounds

Oxmal compounds provided herein comprise at least two or more hydrocarbon-based backbone structures, wherein at least one backbone structure is substituted by at least one  $\alpha,\beta$  unsaturated carboxylic acid or anhydride, and further wherein each backbone structure is linked to one other backbone structure by a bridging group chosen from a direct bond, an ether linkage, or a peroxide linkage located at a non-terminal position of each backbone structure.

The hydrocarbon backbone structure can be chosen from, for example, substituted and unsubstituted straight-chain, branched-chain and polycyclic hydrocarbons. The hydrocarbon backbone structure can be chosen, for example, from fatty acids and rosin acids. The hydrocarbon backbone structure can be chosen from, for example,  $C_{10}$ - $C_{22}$  fatty acids. The hydrocarbon backbone structure can be chosen from, for example,  $C_{16}$ - $C_{22}$  fatty acids. The hydrocarbon backbone structure can be chosen from, for example,  $C_{16}$ - $C_{18}$  fatty acids. The hydrocarbon backbone structure can be, for example, a  $C_{18}$  fatty acid. The hydrocarbon backbone structure can be chosen from, for example, oleic, linoleic, and linolenic acid.

In some embodiments, the hydrocarbon-backbone structure is chosen from polyolefin oligomers having at least one reactive allylic site. In some embodiments, polyolefin oligomers have at least one site of unsaturation. In some embodiments, polyolefin oligomers have at least two sites of unsaturation. In some embodiments, polyolefin oligomers have at least three sites of unsaturation. In some embodiments, the polyolefin oligomers have from 10 to 24 carbons and at least one site of unsaturation. In some embodiments, polyolefin oligomers have from 10 to 24 carbons and from one to five sites of unsaturation. In some embodiments, polyolefin oligomers have from 10 to 24 carbons and from one to three sites of unsaturation. In some embodiments, the polyolefin oligomers have from 16-18 carbons and from one to three sites of unsaturation. In some embodiments, the polyolefin oligomers have 16 or 18 carbons and two sites of unsaturation. In some embodiments, the hydrocarbon-backbone structure could be chosen from non-natural fatty acids, for example fatty acids having odd chain lengths, or 14 carbon chain lengths. In some embodiments, the hydrocarbon-backbone structures chosen

25 from non-natural fatty acids comprise from 1 to 3 sites of unsaturation, for example 2, or for example 3 sites of unsaturation.

In some embodiments, the  $\alpha,\beta$  unsaturated carboxylic acid or anhydride is a synthetic  $\alpha,\beta$  unsaturated carboxylic acid or anhydride. Non-limiting examples of synthetic  $\alpha,\beta$  unsaturated carboxylic acids or anhydrides include maleic anhydride, fumaric acid, and (meth)acrylic acid. In some embodiments, the  $\alpha,\beta$  unsaturated carboxylic acid or anhydride can be a biogenically derived  $\alpha,\beta$  unsaturated carboxylic acid or anhydride. Non-limiting examples of biogenically derived  $\alpha,\beta$  unsaturated carboxylic acids or anhydrides include itaconic acid, itaconic anhydride, aconitic acid, aconitic anhydride, acrylic acid, methacrylic acid, citraconic acid, citraconic anhydride, itaconic acid, mesaconic acid, muconic acid, glutaconic acid, methylglutaconic acid, traumatic acid, and fumaric acid. The acids and anhydrides include any isomers (e.g., enantiomers, diastereomers, and cis-/trans-isomers), and salts. In some embodiments, the  $\alpha,\beta$  unsaturated carboxylic acid or anhydride can be maleic anhydride, fumaric acid, or (meth)acrylic acid.

In certain embodiments all of the hydrocarbon-based backbone structures of an oxmal compound are maleated. In other embodiments, only some, for example, only one of the hydrocarbon-based backbone structures of an oxmal compound are maleated. In some embodiments, two of the hydrocarbon-based backbone structures of an oxmal compound are maleated. In some embodiments, at least one of the hydrocarbon-based backbone structures of an oxmal compound is maleated.

Oxmal compounds within the scope of the invention include oxidized and maleated unsaturated fatty acid compounds of Formula VI:



65 wherein L is chosen from a direct bond,  $—O—$ , or  $—OO—$ ; n is a number chosen from 0, 1, 2, 3, 4, and 5; and R' is a compound of Formula VII:



wherein a, b, c, d, and e are independently a number from 0 to 20; w, x, y, and z are independently 0 or 1; R<sup>1</sup>-R<sup>10</sup> are each independently chosen from L, H, alkyl, alkenyl, alkynyl, alkoxy, amino, hydroxy, and X; wherein at least one of R<sup>1</sup>-R<sup>10</sup> is X; and wherein at least one of R<sup>1</sup>-R<sup>10</sup> is L; wherein X is an  $\alpha,\beta$  unsaturated carboxylic acid or anhydride; wherein the sum of a, b, c, d, e, w, x, y, and z is a number from 8 to 22; and wherein at least one of w, x, y, and z is 1. In some embodiments, the sum of a, b, c, d, e, w, x, y, and z is a number from 12 to 18, while in other embodiments, the sum of a, b, c, d, e, w, x, y, and z is 16. In some embodiments, X is chosen from maleic anhydride, fumaric acid, and (meth)acrylic acid. In some embodiments, X is chosen from



In some embodiments, n is 0 or 1. In some embodiments each R' does not require a substitution with X to be present as long as at least one of R' in the compound of Formula VI does contain at least one X.

In some embodiments, the oxmal compounds have two or three hydrocarbon-based backbone structures (for example, two or three R' structures of Formula VII), and each of the hydrocarbon-based backbone structures is of the same type. For example, without limitation, each of the two or three hydrocarbon-based backbone structures can be a fatty acid. In some embodiments, the oxmal compounds comprise two or three hydrocarbon-based backbone structures, wherein each of the hydrocarbon-based backbone structures is the same. Formulas 8-10, 14-16, 20-22, 29, and 30 below are examples of oxmal compounds having backbone structures chosen from the same fatty acid. Non-limiting examples of oxidized and maleated fatty acids having two hydrocarbon-based

10 backbone structures that are the same include: oxidized and maleated decenoic acid; oxidized and maleated dodecenoic acid; oxidized and maleated cis-9-tetradecenoic acid; oxidized and maleated cis-9-hexadecenoic acid; oxidized and maleated oleic acid; oxidized and maleated linoleic acid; oxidized and maleated linolenic acid; oxidized and maleated cis-6,cis-9,cis-12,cis-15-octadecatetraenoic acid; oxidized and maleated ricinoleic acid; oxidized and maleated cis-9-eicosenoic acid; oxidized and maleated cis-11-eicosenoic acid; oxidized and maleated eicosadienoic acid; oxidized and maleated eicosatrienoic acid; oxidized and maleated arachidonic acid; oxidized and maleated erucic acid; oxidized and maleated docosadienoic acid; oxidized and maleated 4,8,12,15,19-docosapentaenoic acid; oxidized and maleated docosahexaenoic acid; and oxidized and maleated tetracosenoic acid.

20 In some embodiments, the oxmal compounds have two different hydrocarbon-based backbone structures. For example, without limitation, one of the hydrocarbon-based structures can be chosen from fatty acids and one can be chosen from rosin acids. Formulas 11-13, 17-19, and 23-25 below are examples of oxmal compounds having one rosin acid hydrocarbon-based backbone structure and one fatty acid hydrocarbon-based structure. As another non-limiting example, the hydrocarbon backbone-structures can be two different fatty acids. For example, without limitation, one of the hydrocarbon-based backbone structures can be oleic acid and one of the hydrocarbon-based backbone structures can be linoleic acid.

25 In some embodiments, an oxmal compound may be in a salt form. For example, all or some portion of an oxmal compound in an oxmal composition can be in a salt form. In some embodiments, an oxmal compound is in an anionic form. Any suitable counter cation may be used with an anionic oxmal compound, such as Li<sup>+</sup>, K<sup>+</sup>, and Na<sup>+</sup>. In some embodiments, the counter cation is Na<sup>+</sup>. See Example 9.

30 Non-limiting specific structure examples of oxmal compounds in accordance with the invention are illustrated as Formulas 8-32 below. These examples illustrate one isomeric form; other isomers (e.g., cis and trans isomers) can be prepared and accordingly are within the scope of the invention.



**15**-continued  
(IX)

(XI)

**16**

(X)



(XII)



(XIV)



(XV)



(XVI)



17

-continued  
(XVII)



(XIX)



(XXI)



(XXIII)



18

(XVIII)



(XX)



(XXII)



(XXIV)



19

20

-continued  
(XXV)

(XXVI)



(XXVII)



(XXVIII)



(XXIX)



(XXX)



(XXXI)



-continued

(XXXII)



### C. Oxidized Fatty Acid Compositions

Oxidized fatty acid compositions provided herein comprise one or more oxidized fatty acid compounds, wherein when the composition comprises more than one oxidized fatty acid compound, the oxidized fatty acid compounds can be the same or different. Non-limiting examples of oxidized fatty acid compositions, are compositions comprising one or more of the oxidized fatty acid compounds disclosed above, such as compositions containing one or more of oxidized decenoic acid; oxidized dodecenoic acid; oxidized cis-9-tetradecenoic acid; oxidized cis-9-hexadecenoic acid; oxidized oleic acid; oxidized linoleic acid; oxidized linolenic acid; oxidized cis-6,cis-9,cis-12,cis-15-octadecatetraenoic acid; oxidized ricinoleic acid; oxidized cis-9-eicosenoic acid; oxidized cis-11-eicosenoic acid; oxidized eicosadienoic acid; oxidized eicosatrienoic acid; oxidized arachidonic acid; oxidized eicosapentaenoic acid; oxidized erucic acid; oxidized docosadienoic acid; oxidized 4,8,12,15,19-docosapentaenoic acid; oxidized docosahexaenoic acid; and oxidized tetracosenoic acid. In some embodiments, an oxmal composition comprises one or more of oxidized oleic acid; oxidized linoleic acid; oxidized linolenic acid; oxidized cis-9-eicosenoic acid; and oxidized cis-11-eicosenoic acid. In another embodiment, the composition has one or more of oxidized oleic acid; oxidized linoleic acid; and oxidized linolenic acid. In a further embodiment, the composition includes oxidized oleic acid. In a further embodiment, the composition includes one or more compounds of Formulas 1-5 (see, e.g., Example 2).

In some embodiments, the oxidized fatty acid compositions are a source of fatty acids and mixtures of fatty acids that have been oxidized. Sources of fatty acids can be, for example, any natural or synthetic oil, including algal produced and microbial produced oil, that includes at least one site of unsaturation. In certain cases, the distillation products or distillation residues of such oils can serve as the source of fatty acids (e.g. distilled tall oil and tall oil distillation bottoms). In some embodiments, the natural or synthetic oil includes one site of unsaturation, two sites of unsaturation, or more. In some embodiments, the natural or synthetic oil includes at least one site of unsaturation. In some embodiments, the natural or synthetic oil comprises fatty acids having from 10 to 24 carbons and at least one site of unsaturation. In some embodiments, the natural or synthetic oil comprises a fatty acid having from 16 to 22 carbons and from one to five sites of unsaturation. In some embodiments, the natural or synthetic oil comprises a fatty acid having from 16 to 22 carbons and from one to three sites of unsaturation. In some embodiments, the natural or synthetic oil comprises a fatty

acid having 18 carbons and two sites of unsaturation. In other embodiments, these oils can contain a fatty acid having 14 carbons and three sites of unsaturation. In some embodiments, these oils can contain a mixture of fatty acids and rosin acids. In some embodiments, these oils can contain as one significant constituent, linoleic acid, an unsaturated long chain fatty acid, and may also contain other unsaturated fatty acids and rosin acids. In another embodiment, these oils can contain as one significant constituent, oleic acid.

Natural sources of fatty acids, include plant- or animal-based oil compositions. For example, plant- and animal-based oils having unsaturated fatty acids which can be oxidized to produce oxidized fatty acid compositions according to the invention. Depending on the level of oxidation, the compositions may also include unreacted or partially reacted species such as free fatty acid. Non-limiting examples of plant- and animal-based oils include: canola oil; castor oil; coco butter; coconut oil; corn oil; cotton seed oil; crambe oil; linseed oil; olive oil; palm kernel oil; palm oil; peanut oil; rape seed oil; safflower oil; soybean oil; sunflower seed oil; tall oil; tung oil; butter; lard; tallow; yellow grease; and fish oil (e.g., herring oil, menhaden oil, and sardine oil). Oils can be oxidized directly, or if present in a combined form such as triglycerides, can be saponified to their component fatty acids prior to oxidation. In certain embodiments, the source of fatty acids is a plant- or animal-based oil chosen from fish oil, corn oil, soybean oil, and tall oil.

In certain embodiments, the source of fatty acids is a plant-based oil chosen from tall oils and tall oil products. In some embodiments, the tall oil products are oxidized tall oil products. More generally, non-limiting examples of tall oil sources of fatty acids include various tall oil products such as without limitation a tall oil itself, crude tall oil, distilled tall oil products, tall oil fatty acid (TOFA), tall oil distillation bottoms, and specialty tall oil products such as those provided by Georgia-Pacific Chemicals LLC, Atlanta, Ga. For example, tall oil distillation products having greater than about 90% tall oil fatty acid and less than about 6% rosin acid, such as XTOL® 100, XTOL® 101, XTOL® 300, and XTOL® 304; tall oil distillation products such as XTOL® 520, XTOL® 530 and XTOL® 542; tall oil distillation products having at least about 90% rosin acid and less than about 5% tall oil fatty acid, such as LYTOR® 100; oxidized crude tall oil compositions, such as XTOL® MTO; and blends thereof. In some embodiments, such as when the tall oil product is purchased as an oxidized tall oil product, the product may be used without further modification.

Sources of fatty acids can include various amounts of the fatty acids, including various amounts of different fatty acids. In some embodiments, a source of fatty acid can also include rosin acid. For example, TOFA can contain oleic acid, linoleic acid, and linolenic acid, as well as rosin acids, such as abietic and pimamic acid. In some cases, the compositions may further include unsaponifiables or neutral compounds, such as hydrocarbons, higher alcohols, and sterols.

In certain embodiments, a blend of tall oil fatty acid and rosin acid can be used as the source of fatty acids to be oxidized. Such a blend can contain, for example, from about 20% to 99% tall oil fatty acid (e.g., 20%, 25%, 30%, 45%, 50%, 60%, 75%, 82%, 90%, and 99%). In some embodiments, a blend can further contain about 1% to about 55% rosin acid (e.g., 1%, 2.5%, 5%, 10%, 15%, 20%, 25%, 30%, 40%, 50%, and 55%). In some embodiments a blend can contain about 45% to about 90% tall oil fatty acid. In some embodiments a blend can contain about 30% tall oil fatty acid and about 30% rosin acid. In another embodiment, the ratio of tall oil fatty acid to rosin acid can be from about 3:2 to about 4:1 (e.g., 3:2, 4:2, 3:1, and 4:1).

As one non-limiting example, the oxidized fatty acid composition can be a crude tall oil composition that has been oxidized. As another non-limiting example, the oxidized fatty acid composition can be a tall oil fatty acid (TOFA) composition that has been oxidized.

In some embodiments, the oxidized fatty acid composition is an oxidized tall oil product. As one non-limiting example, the oxidized fatty acid composition is a XTOL® MTO.

In some embodiments, an oxidized fatty acid composition can have one or more oxidized fatty acid compounds which are in a salt form. Without being bound by theory, a salt form of an oxidized fatty acid compound can increase the aqueous solubility of the oxidized fatty acid compound. In some embodiments, at least about 10% (e.g., at least about 15%, at least about 20%, at least about 25%, at least about 30%, at least about 35%, at least about 40%, at least about 45%, at least about 50%, at least about 55%, at least about 60%, at least about 70%, at least about 75%, at least about 80%, at least about 85%, at least about 90%, and at least about 95%) of the oxidized fatty acid compounds in an oxidized fatty acid composition can be in a salt form. In some embodiments, at least about 30% of the oxidized fatty acid compounds in an oxidized fatty acid composition can be in a salt form.

In another embodiment, an oxidized fatty acid composition can include an acid compound having at least a first backbone and a second backbone linked by a linking group. The linking group can be a direct bond, an ether linkage, or a peroxide linkage.

In certain embodiments, an oxidized fatty acid composition can include compounds having at least two acid functionalities (e.g., two, three, four, five, six, seven, eight, nine, ten, eleven, or twelve acid functionalities). In some embodiments, an oxidized fatty acid composition can include compounds having at least three acid functionalities. An acid functionality includes anhydrides which can hydrolyze to form acids.

An oxidized fatty acid composition can be characterized by its acid value. As used herein, an "acid value" is the mass of potassium hydroxide (KOH) in milligrams that is required to neutralize one gram of an oxidized fatty acid composition. The acid value can be used as a measure of the amount of carboxylic acid groups in an oxidized fatty acid composition. In a typical procedure, a known amount of an oxidized fatty acid composition is dissolved in organic solvent and is titrated with a solution of potassium hydroxide of known concentration. The acid value can be determined by using a potassium

hydroxide solution that contains phenolphthalein as a color indicator or using potentiometric analysis. Standard methods used for determining acid value are ASTM D 465-05 and AOC S Te 1a-64.

In some embodiments, the acid value can be from about 50 mg KOH/g to about 200 mg KOH/g (e.g., 60 mg KOH/g; 80 mg KOH/g, 100 mg KOH/g; 120 mg KOH/g; 150 mg KOH/g; 160 mg KOH/g; 170 mg KOH/g; 180 mg KOH/g; and 200 mg KOH/g). In some embodiments, the acid value can be from about 80 mg KOH/g to about 200 mg KOH/g. In some embodiments, the acid value can be from about 100 mg KOH/g to about 180 mg KOH/g. In certain embodiments, the acid value can range from about 120 mg KOH/g to about 150 mg KOH/g. In other embodiments, the acid value is about 130 mg KOH/g. In some embodiments, the acid value is at least about 80 mg KOH/g. In some embodiments, the acid value is at least about 110 mg KOH/g.

Viscosity of an oxidized fatty acid composition is another method of characterizing these compositions. Without being bound by theory, the viscosity of an oxidized fatty acid composition increases, compared to the viscosity of the starting composition, with an increase in acid functionality, e.g., the number of acid groups or groups, such as anhydrides which can hydrolyze to form acids. Both a Gardner-Holdt and a Brookfield Viscosity value can be used to characterize an oxidized fatty acid composition. An apparent viscosity can be determined using a Brookfield viscometer. This measures the torque required to rotate a spindle at constant speed in a solution of an oxidized fatty acid composition at 25° C. Standard test methods used for measuring Brookfield viscosity are ASTM D 803-03 and AOCS Ja 10-87 (93). In certain embodiments, the viscosity range for the oxidized fatty acid products can range from about 1000 to about 6000 cPs at 25° C. In some embodiments, the viscosity range for the oxidized fatty acid products can range from about 1300 to about 5000 cPs at 25° C. In some embodiments, the viscosity range for the oxidized fatty acid products can range from about 3000 to about 4000 cPs at 25° C. Standard test methods for determining Gardner-Holdt viscosity are ASTM D1545-07 and AOCS Ja 11-87 (93).

In some embodiments, the oxidized fatty acid compositions described above can be oxidized clean fatty acid compositions as defined herein.

#### D. Oxmal Compositions

Oxmal compositions provided herein comprise one or more oxmal compounds, wherein when the composition comprises more than one oxmal compound, the oxmal compounds can be the same or different. Non-limiting examples of oxmal compositions, are compositions comprising one or more of the oxmal compounds disclosed above, such as compositions containing one or more of oxidized and maleated decenoic acid; oxidized and maleated dodecenoic acid; oxidized and maleated cis-9-tetradecenoic acid; oxidized and maleated cis-9-hexadecenoic acid; oxidized and maleated oleic acid; oxidized and maleated linoleic acid; oxidized and maleated linolenic acid; oxidized and maleated cis-6,cis-9, cis-12,cis-15-octadecatetraenoic acid; oxidized and maleated ricinoleic acid; oxidized and maleated cis-9-eicosenoic acid; oxidized and maleated cis-11-eicosenoic acid; oxidized and maleated eicosadienoic acid; oxidized and maleated eicosatrienoic acid; oxidized and maleated arachidonic acid; oxidized and maleated eicosapentaenoic acid; oxidized and maleated erucic acid; oxidized and maleated docosadienoic acid; oxidized and maleated 4,8,12,15,19-docosapentaenoic acid; oxidized and maleated docosahexaenoic acid; and oxidized and maleated tetraicosenoic acid. In some embodiments, an oxmal composition comprises one or more of oxi-

dized and maleated oleic acid; oxidized and maleated linoleic acid; oxidized and maleated linolenic acid; oxidized and maleated cis-9-eicosenoic acid; and oxidized and maleated cis-11-eicosenoic acid. In another embodiment, the composition has one or more of oxidized and maleated oleic acid; oxidized and maleated linoleic acid; and oxidized and maleated linolenic acid. In a further embodiment, the composition includes oxidized and maleated oleic acid. In a further embodiment, the composition includes one or more compounds of Formulas 8-32.

In some embodiments, the oxmal compositions are a source of fatty acids, rosin acids, and mixtures of fatty acids and rosin acids that have been oxidized and/or maleated. Sources of fatty acids, rosin acids, and mixtures thereof, can be, for example, any natural or synthetic oil, including algal produced and microbial produced oil, that includes at least one site of unsaturation. In certain cases, the distillation products or distillation residues of such oils can serve as the source of fatty acids, rosin acids, and mixtures thereof (e.g. distilled tall oil and tall oil distillation bottoms). In some embodiments, the natural or synthetic oil includes one site of unsaturation, two sites of unsaturation, or more. In some embodiments, the natural or synthetic oil includes at least one site of unsaturation. In some embodiments, the natural or synthetic oil comprises from 10 to 24 carbons and at least one site of unsaturation. In some embodiments, the natural or synthetic oil comprises from 16 to 22 carbons and from one to five sites of unsaturation. In some embodiments, the natural or synthetic oil comprises from 16 to 22 carbons and from one to three sites of unsaturation. In some embodiments, the natural or synthetic oil comprises 18 carbons and two sites of unsaturation. In other embodiments, these oils can contain a fatty acid having 14 carbons and three sites of unsaturation. In some embodiments, these oils can contain as one significant constituent, linoleic acid, an unsaturated long chain fatty acid, and may also contain other unsaturated fatty acids and rosin acids. In another embodiment, these oils can contain as one significant constituent, oleic acid.

Natural sources of fatty acids, rosin acids, and mixtures thereof, include plant- or animal-based oil compositions. For example, plant- and animal-based oils having double bonds, i.e., sites of unsaturation in their hydrocarbon chains can be oxidized and maleated to produce oxmal compositions according to the invention. Depending on the level of maleation, the compositions may also include unreacted or partially reacted species such as free fatty acid and rosin acid, maleated but not oxidized fatty acid and rosin acid, oxidized but not maleated fatty acid and rosin acid, and oxidized and partially maleated fatty acid and rosin acid. Non-limiting examples of plant- and animal-based oils include: canola oil; castor oil; coco butter; coconut oil; corn oil; cotton seed oil; crambe oil; linseed oil; olive oil; palm kernel oil; palm oil; peanut oil; rape seed oil; safflower oil; soybean oil; sunflower seed oil; tall oil; tung oil; butter; lard; tallow; yellow grease; and fish oil (e.g., herring oil, menhaden oil, and sardine oil). Oils can be oxidized and/or maleated directly, or if present in a combined form such as triglycerides, can be saponified to their component fatty acids before the oxidation and/or maleation reactions.

In certain embodiments, the source of fatty acids, rosin acids, and/or mixtures thereof is a plant- or animal-based oil chosen from fish oil, corn oil, soybean oil, and tall oil.

In certain embodiments, the source of fatty acids, rosin acids, and/or mixtures thereof is a plant-based oil chosen from tall oils and tall oil products. In some embodiments, tall oil products are maleated tall oil products. In some embodiments, the tall oil products are oxidized tall oil products. More

generally, non-limiting examples of tall oil sources of fatty acids, rosin acids, and mixtures thereof include various tall oil products such as without limitation a tall oil itself, crude tall oil, distilled tall oil products, tall oil fatty acid (TOFA), TOFA which has been maleated in a range of from about 6% to about 25%, rosin acids, tall oil distillation bottoms, and specialty tall oil products such as those provided by Georgia-Pacific Chemicals LLC, Atlanta, Ga. For example, tall oil distillation products having greater than about 90% tall oil fatty acid and less than about 6% rosin acid, such as XTOL® 100, XTOL® 101, XTOL® 300, and XTOL® 304; tall oil distillation products such as XTOL® 520, XTOL® 530 and XTOL® 542; tall oil distillation products having at least about 90% rosin acid and less than about 5% tall oil fatty acid, such as LYTOR® 100; tall oil blends of tall oil fatty acid distillation bottoms and a distilled tall oil, which blend has been maleated, such as XTOL® 690, XTOL® 692; oxidized crude tall oil compositions, such as XTOL® MTO; and blends thereof.

Sources of fatty acids, rosin acids, and mixtures thereof can include various amounts of the fatty acids, rosin acids, and mixtures thereof, including various amounts of different fatty acids and rosin acids. For example, TOFA can contain oleic acid, linoleic acid, and linolenic acid, as well as rosin acids, such as abietic and pimamic acid. In some cases, the compositions may further include unsaponifiables or neutral compounds, such as hydrocarbons, higher alcohols, and sterols when using certain tall oil fractions.

In certain embodiments, a blend of tall oil fatty acid and rosin acid can be used as the source of fatty acids and rosin acids (i.e. the source of hydrocarbon-based backbone structures) to be oxidized and maleated. Such a blend can contain, for example, from about 20% to 99% tall oil fatty acid (e.g., 20%, 25%, 30%, 45%, 50%, 60%, 75%, 82%, 90%, and 99%) and about 1% to about 55% rosin acid (e.g., 1%, 2.5%, 5%, 10%, 15%, 20%, 25%, 30%, 40%, 50%, and 55%). In some embodiments a blend can contain about 45% to about 90% tall oil fatty acid. In some embodiments a blend can contain about 30% tall oil fatty acid and about 30% rosin acid. In another embodiment, the ratio of tall oil fatty acid to rosin acid can be from about 3:2 to about 4:1 (e.g., 3:2, 4:2, 3:1, and 4:1).

As one non-limiting example, the oxmal composition can be a crude tall oil composition that has been oxidized and maleated (see Example 5). As another non-limiting example, the oxmal composition can be a tall oil fatty acid (TOFA) composition that has been oxidized and maleated (see Example 6).

In some embodiments, the oxmal compositions are a source of maleated tall oil product that has been oxidized. As one non-limiting example, the oxmal composition is a XTOL® 690 that has been oxidized (see Example 3). As another non-limiting example, the oxmal composition is a XTOL® 692 that has been oxidized (see Example 3).

In some embodiments, the oxmal composition is a source of oxidized tall oil product that has been maleated. As one non-limiting example, the oxmal composition is a XTOL® MTO that has been maleated (see Example 4).

In some embodiments, an oxmal composition can have one or more oxmal compounds which are in a salt form. Without being bound by theory, a salt form of an oxmal compound can increase the aqueous solubility of the oxmal compound. In some embodiments, at least about 10% (e.g., at least about 15%, at least about 20%, at least about 25%, at least about 30%, at least about 35%, at least about 40%, at least about 45%, at least about 50%, at least about 55%, at least about 60%, at least about 70%, at least about 75%, at least about 80%, at least about 85%, at least about 90%, and at least about

95%) of the oxmal compounds in an oxmal composition can be in a salt form. In some embodiments, at least about 30% of the oxmal compounds in an oxmal composition can be in a salt form.

In another embodiment, an oxmal composition can include an acid compound having at least a first backbone and a second backbone linked by a linking group. The linking group can be a direct bond, an ether linkage, or a peroxide linkage. In some embodiments, the first and second backbone can be independently chosen from a maleated unsaturated fatty acid or maleated rosin acid. In some embodiments, the first backbone is chosen from a maleated unsaturated fatty acid or maleated rosin acid and the second backbone is chosen from an unsaturated fatty acid or rosin acid.

Non-limiting examples of maleated unsaturated fatty acids can include: maleated decenoic acid; maleated dodecenoic acid; maleated cis-9-tetradecenoic acid; maleated cis-9-hexadecenoic acid; maleated oleic acid; maleated linoleic acid; maleated linolenic acid; maleated cis-6,cis-9,cis-12,cis-15-octadecatetraenoic acid; maleated ricinoleic acid; maleated cis-9-eicosenoic acid; maleated cis-11-eicosenoic acid; maleated eicosadienoic acid; maleated eicosatrienoic acid; maleated arachidonic acid; maleated eicosapentaenoic acid; maleated erucic acid; maleated docosadienoic acid; maleated 4,8,12,15,19-docosapentaenoic acid; maleated docosahexaenoic acid; and maleated tetracosenoic acid.

In certain embodiments, the maleated unsaturated fatty acid is maleated oleic acid; maleated linoleic acid; maleated linolenic acid; maleated cis-9-eicosenoic acid; or maleated cis-11-eicosenoic acid. In another embodiment, the maleated unsaturated fatty acid is maleated oleic acid; maleated linoleic acid; and maleated linolenic acid. In a further embodiment, the maleated unsaturated fatty acid is maleated oleic acid.

In certain embodiments, an oxmal composition can include compounds having at least three acid functionalities (e.g., three, four, five, six, seven, eight, nine, ten, eleven, or twelve acid functionalities). In some embodiments, an oxmal composition can include compounds having at least six acid functionalities. An acid functionality includes anhydrides which can hydrolyze to form acids.

In certain embodiments, the oxmal composition can be maleated from about 2% to about 40% by weight (e.g., 2%, 3.5%, 5%, 6%, 7.5%, 8%, 10%, 12%, and 15%). In some embodiments, the percent maleation is from about 2% to about 25% by weight. In one embodiment, the percent maleation is 3.5% by weight, while in another embodiment, the percent maleation is 12% by weight. In some embodiments, the percent maleation is 5% by weight. In some embodiments, the percent maleation is 6% by weight. The composition of products prepared is related to the percent maleation performed. Accordingly, in some oxmal compositions, oxmal compounds may include compounds that have been maleated, for example, on at least one hydrocarbon-based backbone structure, at least two hydrocarbon-based backbone structures, on all hydrocarbon-based backbone structures. In certain embodiments, an oxmal composition may further comprise compounds that have been oxidized but have not been maleated.

An oxmal composition can be characterized by its acid value. As used herein, an "acid value" is the mass of potassium hydroxide (KOH) in milligrams that is required to neutralize one gram of an oxmal composition. The acid value can be used as a measure of the amount of carboxylic acid groups in an oxmal composition. In a typical procedure, a known amount of an oxmal composition is dissolved in organic solvent and is titrated with a solution of potassium hydroxide of

known concentration. The acid value can be determined by using a potassium hydroxide solution that contains phenolphthalein as a color indicator or using potentiometric analysis. Standard methods used for determining acid value are

5 ASTM D 465-05 and AOCS Te 1a-64.

In some embodiments, the acid value can be from about 50 mg KOH/g to about 400 mg KOH/g (e.g., 65 mg KOH/g; 100 mg KOH/g; 150 mg KOH/g, 200 mg KOH/g; 250 mg KOH/g; 330 mg KOH/g; and 400 mg KOH/g). In some embodiments, 10 the acid value can be from about 150 mg KOH/g to about 300 mg KOH/g. In some embodiments, the acid value can be from about 150 mg KOH/g to about 225 mg KOH/g. In certain embodiments, the acid value can range from about 200 mg KOH/g to about 300 mg KOH/g. In other embodiments, the acid value is about 200 mg KOH/g.

Viscosity of an oxmal composition is another method of characterizing these compositions. Without being bound by theory, the viscosity of an oxmal composition increases, compared to the viscosity of the starting composition, with an increase in acid functionality, e.g., the number of acid groups or groups, such as anhydrides which can hydrolyze to form acids. Both a Gardner-Holdt and a Brookfield Viscosity value can be used to characterize an oxmal composition. An apparent viscosity can be determined using a Brookfield viscometer. This measures the torque required to rotate a spindle at constant speed in a solution of an oxmal composition at 25° C. Standard test methods used for measuring Brookfield viscosity are ASTM D 803-03 and AOCS Ja 10-87 (93). In certain 20 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790

In some embodiments, the composition can comprise animal oil fatty acids, plant oil fatty acids, algal oil fatty acids, microbially derived fatty acids, and mixtures thereof.

In some embodiments, oxidation is accomplished by heating the compositions containing the fatty acid backbone structures, such as for example tall oils, in the presence of oxygen or air. Unsaturated fatty acids can be polymerized by heating them in the presence of oxygen or air. This polymerization can cause an increase in the viscosity of the oxidized fatty acid composition. A catalyst can be used to increase the speed of the oxidation reaction in order to reduce the time required to attain the desired level of oxidation and associated viscosity increase, or to reduce the temperature at which the oxidation is conducted. Use of such a catalyst is optional. Without being bound by theory, the oxidative heating treatment is believed to cause crosslinking of the fatty acids via their double bonds (sites of unsaturation) and allylic sites, via a direct bond, an ether linkage, or a peroxide linkage. The oxidation treatment is continued until a desired result is obtained, for example, a desired acid value or a desired viscosity.

In some embodiments, the process of producing an oxidized fatty acid composition involves oxidizing a tall oil composition by heating the tall oil material to a temperature at least about 150° C., for example to a temperature in the range of about 160° C. to about 170° C., followed by sparging oxygen or air through the heated tall oil composition. As understood by those skilled in the art, a variety of techniques and devices can advantageously be used to inject the oxygen or air into the heated tall oil and the present method is not limited to any specific technique or equipment. As discussed above, the oxidation reaction can be continued until the desired acid value or viscosity is achieved in the tall oil, indicative that the desired level of cross-linking has been obtained in the oxidized tall oil material.

In some embodiments, tall oil distillate components suitable for use in the process of making an oxidized fatty acid composition include without limitation: fatty acids, tall oil rosin acids, and mixtures of these fractions. The refinement (i.e. fractionation) of tall oil can, for example, provide C<sub>16</sub>-C<sub>18</sub> saturated and unsaturated fatty acids as well as fatty acid/rosin acid mixtures. In preparing oxidized tall oil, such tall oil distillate components, lighter (i.e. lower boiling) or heavier (i.e. higher boiling) components, or components having broader or narrower boiling point ranges may be used in the reaction. Mixtures or blends of various tall oil distillate fractions may also be employed as the tall oil material. Fatty acid/rosin acid mixtures in a desired ratio may be obtained in a single distillate fraction by adjusting tall oil fractionation conditions. Representative tall oil distillate components include commercially available products XTOL® 100, XTOL® 300, XTOL® 304, and XTOL® 520 (from Georgia-Pacific Chemicals LLC, Atlanta, Ga.).

In one embodiment, for example, a mixture of a first tall oil distillate fraction comprising predominantly tall oil fatty acids (e.g., XTOL® 100) and a second tall oil distillate fraction comprising predominantly rosin acids (e.g., LYTOR® 100) may be blended in a wide range of proportions. In such mixtures, representative amounts of fatty acids and rosin acids range from about 20% to about 99% by weight and from about 1% to about 55% by weight, respectively. Representative weight ratios of the first tall oil distillate fraction to the second tall oil distillate fraction may range from about 3:2 to about 4:1. Depending on the tall oil composition and fractionation conditions, a single tall oil distillate fraction may

also suffice to yield a composition that is substantially the same as any of the blends of tall oil distillate fractions discussed above.

#### B. Preparation of Oxmal Compounds and Compositions

Processes for preparing oxmal compounds and compositions, as described above, are also provided herein. Although the examples and descriptions herein emphasize methods of making compositions, the chemistry is equally applicable to methods of making compounds.

10 In some embodiments, an oxmal compound is prepared by oxidizing and maleating a hydrocarbon-based backbone structure having at least one site of unsaturation and at least one reactive allylic site. The hydrocarbon-backbone based structure can be, for example, a fatty acid, a rosin acid, or a polyolefin oligomer with at least one reactive allylic site. In some embodiments, the hydrocarbon-backbone structure is a C<sub>16</sub> or C<sub>18</sub> fatty acid, such as for example oleic acid, linoleic acid, and linolenic acid. In some embodiments, the backbone structure is first oxidized and then maleated. In some embodiments, the backbone structure is first maleated and then oxidized.

15 In some embodiments, an oxmal composition is prepared by the process of: (a) maleating a composition comprising one or more hydrocarbon-based backbone structures having at least one site of unsaturation; and (b) oxidizing the composition. In some embodiments, step (a) is performed before step (b), while in other embodiments, step (b) is performed before step (a). In some embodiments, the composition can comprise (i.e. the hydrocarbon-based backbone structures are) fatty acids, rosin acids, distillation products thereof, or mixtures thereof. In some embodiments, the compositions are chosen from tall oil, animal oils, plant oils, algal produced oils, microbial produced oils, distillation products thereof, and mixtures thereof. A person of ordinary skill will appreciate that certain of these oils or products thereof may have to be saponified prior to oxidation and maleation to obtain an appropriate backbone structure, or a fatty acid.

20 In some embodiments, suitable oils which can be used for preparing an oxidized and maleated composition include without limitation: linseed (flaxseed) oil, castor oil, tung oil, soybean oil, cottonseed oil, olive oil, canola oil, corn oil, sunflower seed oil, coconut oil, rape seed oil, safflower oil, tall oil, palm oil, the distillation products thereof, and mixtures thereof. These oils contain as one constituent linoleic acid, an unsaturated long chain fatty acid as well as other unsaturated fatty acids. In some embodiments, suitable oils include without limitation fish oil, such as herring oil, menhaden oil, and sardine oil.

25 In some embodiments, the compositions can comprise animal oil fatty acids, plant oil fatty acids, algal oil fatty acids, microbially derived fatty acids, and mixtures thereof.

30 In the preparation of an oxmal composition, as with the preparation of an oxmal compound, the oxidation and the maleation of the hydrocarbon-backbone structures of the composition can be conducted in either order. For example, a fatty acid composition can first be maleated and then the maleation can be followed by an oxidation (see Example 4 and 5). Alternatively, the fatty acid composition can first be oxidized and then the oxidized composition can be maleated (see Example 3).

35 In some embodiments, the process of making an oxmal composition comprises oxidizing a commercially available maleated fatty acid composition, such as without limitation XTOL® 690 or XTOL® 692. In some embodiments, the process of making an oxmal composition comprises maleating a commercially available oxidized tall oil composition, such as without limitation XTOL® MTO.

31

In some embodiments, oxidation is accomplished by heating the compositions containing the hydrocarbon-backbone based structures, such as for example tall oils, in the presence of oxygen or air. Unsaturated hydrocarbon-based structures can be polymerized by heating them in the presence of oxygen or air. This polymerization can cause an increase in the viscosity of the oxmal composition. A catalyst can be used to increase the speed of the oxidation reaction in order to reduce the time required to attain the desired level of oxidation and associated viscosity increase, or to reduce the temperature at which the oxidation is conducted. Use of such a catalyst is optional. In some embodiments, a hydrocarbon-based structure can be a fatty acid, rosin acid, or mixtures thereof. Without being bound by theory, the oxidative heating treatment is believed to cause crosslinking of the hydrocarbon chains acid via their double bonds (sites of unsaturation) and allylic sites, via a direct bond, an ether linkage, or a peroxide linkage. The oxidation treatment is continued until a desired result is obtained, for example, a desired acid value or a desired viscosity.

In some embodiments, the oxidation step in the process of producing an oxmal composition involves oxidizing a tall oil composition by heating the tall oil material to a temperature at least about 150° C., for example to a temperature in the range of about 160° C. to about 170° C., followed by sparging oxygen or air through the heated tall oil composition. As understood by those skilled in the art, a variety of techniques and devices can advantageously be used to inject the oxygen or air into the heated tall oil and the present method is not limited to any specific technique or equipment. As discussed above, the oxidation reaction can be continued until the desired acid value or viscosity is achieved in the tall oil, indicative that the desired level of cross-linking has been obtained in the oxidized tall oil material.

In some embodiments, the maleation step in the process of producing an oxmal composition involves reaction of the hydrocarbon-based structures in the composition with one or more  $\alpha,\beta$  unsaturated carboxylic acids or anhydrides. The amount of  $\alpha,\beta$  unsaturated carboxylic acid or anhydride used varies based on the composition to be maleated. Suitable amounts of the anhydride (or acid(s)) may range from about 2% to about 40% by weight, based on the combined weight of the composition and the anhydride (or acid(s)) and/or the desired amount of maleation. In some embodiments, the amount of anhydride (or acid(s)) can range from about 2% to about 25% by weight, usually from about 2% to about 15% by weight, based on the combined weight of the composition and the anhydride (or acid(s)) and/or the desired amount of maleation. In some embodiments, the  $\alpha,\beta$  unsaturated carboxylic acid or anhydride is chosen from maleic anhydride, fumaric acid, or (meth)acrylic acid. In some embodiments, the  $\alpha,\beta$  unsaturated carboxylic acid or anhydride is a biogenically derived unsaturated carboxylic acid or anhydride. The composition of products prepared is related to the percent maleation performed. Accordingly, in some oxmal compositions, oxmal compounds may include compounds that have been maleated, for example, on at least one hydrocarbon-based backbone structure, at least two hydrocarbon-based backbone structures, or all hydrocarbon-based backbone structures. In certain embodiments, an oxmal composition may further comprise compounds that have been oxidized but have not been maleated.

In contrast to the prior art, where there apparently has been a concerted effort to use tall oil materials containing primarily, if not almost exclusively, tall oil fatty acids (TOFA) and to conduct the maleation reaction (e.g. the reaction with maleic anhydride and/or fumaric acid, and/or acrylic acid), in

32

a way to promote the formation of the Diels-Alder reaction adduct with linoleic acid (generally by using a catalyst), the present inventors have found that such restrictions are not necessary. In some embodiments according to the invention, the conditions under which the maleation reaction proceeds do not need to be controlled (e.g. a catalyst is not needed) such that the Diels-Alder reaction predominates; there is no need to focus on the production of the Diels-Alder reaction adduct with conjugated fatty acids, such as linoleic acid.

For example, the maleation of a tall oil, such as without limitation a crude tall oil or tall oil distillate or component, proceeds by reaction of the tall oil and, for example, one or more of maleic anhydride, fumaric acid, and (meth)acrylic acid. Once combined, the reaction mixture is heated to a temperature of from about 150° C. to about 250° C. In certain embodiments, the reaction temperature is from about 200° C. to about 230° C. In other embodiments, the reaction temperature is from about 215° C. to about 225° C. In some embodiments, a catalyst can be used. Such catalysts are known in the art.

The maleation reaction is essentially complete after a reaction time from about 5 hours to about 36 hours, and typically from about 20 hours to about 30 hours. Without being bound by theory, the maleic anhydride, fumaric acid, and/or (meth) acrylic acid reacts with the hydrocarbon-based material, at the various sites of unsaturation present in the material. For example, the reaction of maleic anhydride with an unsaturated tall oil fatty acid results in the addition of the anhydride ring to the acid at olefinic sites via the so-called "ene" reaction. The reaction of maleic anhydride with a rosin acid derived from tall oil, at diolefinic sites and with conjugated unsaturated fatty acids, may alternatively form a Diels-Alder addition product having a 6-membered ring with one site of unsaturation. Non-limiting examples of representative reactions that can occur are illustrated in U.S. Pat. No. 4,927,669.

A representative set of structures of molecular species potentially found in maleated tall oil compositions (especially tall oil compositions maleated with maleic anhydride) suitable for use as the starting material for making chemically modified oxidized and maleated unsaturated fatty acid compositions include the Diels-Alder reaction product with conjugated linoleic acid and ene reaction products with oleic and elaidic acids as follows:



33



As will be appreciated by those skilled in the art, certain analogous structures are formed when using any  $\alpha,\beta$  unsaturated carboxylic acid or anhydride for these maleation reactions.

In some embodiments, tall oil distillate components suitable for use in the process of making an oxmal composition include without limitation: fatty acids, tall oil rosin acids, and mixtures of these fractions. The refinement (i.e. fractionation) of tall oil can, for example, provide  $C_{16}$ - $C_{18}$  saturated and unsaturated fatty acids as well as fatty acid/rosin acid mixtures. In preparing maleated tall oil, such tall oil distillate components, lighter (i.e. lower boiling) or heavier (i.e. higher boiling) components, or components having broader or narrower boiling point ranges may be used in the reaction with an  $\alpha,\beta$  unsaturated carboxylic acid or anhydride. Mixtures or blends of various tall oil distillate fractions may also be employed as the tall oil material. Fatty acid/rosin acid mixtures in a desired ratio may be obtained in a single distillate fraction by adjusting tall oil fractionation conditions. Representative tall oil distillate components include commercially available products XTOL® 100, XTOL® 300, XTOL® 304, and XTOL® 520 (from Georgia-Pacific Chemicals LLC, Atlanta, Ga.).

In one embodiment, for example, a mixture of a first tall oil distillate fraction comprising predominantly tall oil fatty acids (e.g., XTOL® 100) and a second tall oil distillate fraction comprising predominantly rosin acids (e.g., LYTOR® 100) may be blended in a wide range of proportions. In such mixtures, representative amounts of fatty acids and rosin acids range from about 20% to about 99% by weight and from about 1% to about 55% by weight, respectively. Representative weight ratios of the first tall oil distillate fraction to the second tall oil distillate fraction may range from about 3:2 to about 4:1. If such a blend is used to form a maleated tall oil material via reaction with an  $\alpha,\beta$  unsaturated carboxylic acid or anhydride, suitable amounts of the anhydride (or acid(s)) may range from about 2% to about 25% by weight, usually from about 2% to about 15% by weight, based on the combined weight of the tall oil fractions and the anhydride (or acid(s)). Depending on the tall oil composition and fractionation conditions, a single tall oil distillate fraction may also suffice to yield a composition that is substantially the same as any of the blends of tall oil distillate fractions discussed above.

In certain embodiments, maleated unsaturated fatty acid compositions suitable for use in making an oxidized and maleated unsaturated fatty acid composition are commercially available. For example, maleated tall oil products can be obtained commercially as XTOL® 690 and XTOL® 692 (from Georgia-Pacific Chemicals LLC, Atlanta, Ga.).

34

As noted above, the steps of oxidation and maleation of hydrocarbon-based composition can be conducted in either order, as illustrated by the examples which follow.

#### C. Collector Blends

Compositions for use in the methods described herein can include blends of one or more of the collectors described herein. In some embodiments, the blends can further contain other products suitable for use in a froth flotation cell. In some embodiments, a blend can contain from 1% to 99% of a collector (e.g., 10%, 25%, 30%, 50%, 65%, 80%, 95%, or 99%) and from 1% to 99% of one or more additional components (e.g., 10%, 25%, 30%, 50%, 65%, 80%, 95%, or 99%). In some embodiments, a blend can contain more than one collector. In some embodiments, a blend can be composed of a collector and one or more of a frothing agent, a depressant, an additional collector, an activator, and a modifier, as described above. In some embodiments, a blend contains a collector and a frothing agent. In some embodiments, a blend contains a collector and a depressant. In some embodiments, a blend contains a collector and an activator. In some embodiments, a blend contains a collector and a modifier.

In some embodiments, a blend of an oxidized fatty acid composition and an oxmal composition can be prepared. Such a blend can contain from about 1% to about 99% of an oxidized fatty acid composition and from about 1% to about 99% of an oxmal composition. In some embodiments, a blend contains about 75% of an oxidized fatty acid composition and about 25% of an oxmal composition. In some embodiments, a blend contains about 85% of an oxidized fatty acid composition and about 15% of an oxmal composition.

As described previously, a collector as described herein, e.g., an oxidized fatty acid composition, an oxidized clean fatty acid composition, an oxmal composition, and mixtures thereof, can be blended with various additional components used in the flotation of minerals. A collector and one or more additional components can be readily combined and used under general flotation methods for the flotation of many different mineral species. For example, a composition for use in mineral flotation can include a collector blended with:

- 40 (1) an alkylsulphosuccinate to float biotite, calcite, dolomite, magnesite, iron oxides, rutile, and ilmenite;
- (2) with an alkyl sulfate to float celestite, gypsum, kainite, anglesite, bauxite, barite, alunite, fluorspar, and anhydrite;
- (3) a mono or diphosphoric acid ester to float biotite, iron oxides, fluorspar, and titanium minerals;
- (4) an oxidized petroleum product to float alunite;
- (5) a non-ionic surfactant, such as an alkoxylated alkylphenol, to float coal, feldspar, apatite, and sulfur;
- (6) crude tall oil, crude tall oil distillation fractions, and mixtures thereof to float coal, feldspar, apatite, and sulfur;
- (7) alkoxylated alkylphenol formaldehyde condensates to float coal, feldspar, apatite, and sulfur;
- (8) a succinic acid ester, succinic acid half ester, and mixtures thereof to float fluorspar and apatite;
- (9) an alkenylsuccinic acid, alkenylsuccinate salt, and mixtures thereof to float scheelite;
- (10) a sarscoside to float apatite and other phosphate ores;
- (11) a vegetable oil, such as rice bran oil, to float apatite and other phosphate ores; and
- (12) an alkyl hydroxamate to float oxide, hydroxide, and phosphate minerals like aeschynite, anatase, bindheimite, bixbyite, brookite, chrysoberyl, columbite, corundum, cuprite, euxenite, fergusonite, hausmannite, hematite, ilmenite, perovskite, periclase, polycrase, pseudobrookite, pyrochlore, betafite, microlite, ramsdellite, romanechite, cassiterite, plattnerite, pyrolusite, rutile, stishovite, samarskite, senarmontite, chromite, franklinite, magnesiochromite, mag-

netite, spinel, taaffeite, tantalite, tapiolite, uraninite, valen-  
tinite, zincite, brucite, gibbsite, goethite, limonite, manga-  
nite, psilomelane, romeite, stetefeldtite, carnotite,  
tyuyamunite, meta-autunite, autunite, apatite, phosphura-  
nylite, tobernite, rhabdophane, triphyllite, woodhouseite, bra-  
zilianite, chirchite, lithiophilite, hinsdalite, svanbergite,  
arthurite, cacoxenite, tsumebite, variscite, hopeite, meta-  
ankoleite, scholzite, strengite, whitlockite, xenotime,  
amblygonite, kidwellite, laueite, meta-uranocircite, meta-  
variscite, montebrasite, pseudomalachite, rockbridgeite,  
strunzite, tarbutite, whiteite, anapite, augelite, beraunite,  
chalcosiderite, collinsite, uranocircite, zeunerite, boltwood-  
ite, uranophane, meta-torbernite, meta-uranocircite,  
walpurgite, zippeite, uranopilitite, coconinoite, monazite,  
Stibiconite, quetzalcoatlite, zincite, hodgkinsonite, aurichal-  
cite, hydrozincite, rosasite, descloizite, Hopeite, veszelyite,  
ktenasite, and gahnite.

An oxidized fatty acid composition, an oxidized clean fatty acid composition, an oxmal composition, and mixtures thereof can also be blended with one or more fatty acids. For example, an oxidized fatty acid composition can be blended with oleic acid.

#### IV. Kits and Articles of Manufacture

The collector compounds and compositions described herein may be packaged as articles of manufacture (e.g., kits) containing packaging material, a collector compound or composition as provided herein within the packaging material, and a label that indicates that the collector compound or composition, is useful for froth flotation.

Typically, a kit includes a collector as described herein. In some embodiments, a kit includes at least two collectors. In some embodiments, a kit includes an oxidized fatty acid composition. In certain embodiments, a kit can include directions for use of the kit (e.g., instructions for froth flotation). In some embodiments, a kit includes an oxmal composition. In some embodiments, a kit includes one or more oxidized fatty acid compositions and one or more oxmal compositions. In some embodiments, the kit further comprises one or more of a frothing agent, a depressant, an additional collector, an activator, a modifier, and mixtures thereof. In certain embodiments, a kit can include a collector and a frothing agent. In another embodiment, a kit can include a collector and a depressant. In some embodiments, a kit can include a collector and an activator. In some embodiments, a kit can include a collector and a modifier. In some embodiments, a kit includes a blend of a collector and one or more of a frothing agent, a depressant, an additional collector, an activator, a modifier, and mixtures thereof.

In some embodiments, the kit can include a collector and a label that indicates that the contents are to be used in froth flotation. In another embodiment, the kit can include a collector and a label that indicates that the contents are to be used in phosphate froth flotation. In another embodiment, the kit can include a collector and a label that indicates that the contents are to be used in potash froth flotation. In a further embodiment, a kit can include a collector and a label that indicates that the contents are to be used in combination with one or more of a frothing agent, a depressant, an additional collector, an activator, a modifier, and mixtures thereof.

In one embodiment, the present invention is:

1. A method of froth flotation, the method comprising floating a mineral using a collector comprising one or more of an oxidized clean fatty acid composition, an oxmal composition, and mixtures thereof.
2. A method according to paragraph 1, wherein the collector is an anionic collector.

3. A method according to paragraph 2, wherein the anionic collector has a counter cation chosen from  $\text{Li}^+$ ,  $\text{Na}^+$ ,  $\text{K}^+$ ,  $\text{NH}_4^+$ , alkyl ammonium ions, and imidazoline cations.
4. A method according to paragraph 2, wherein the anionic collector has a counter cation chosen from  $\text{Li}^+$ ,  $\text{Na}^+$ , and  $\text{K}^+$ .
5. A method according to any of the preceding paragraphs, wherein the collector is an oxidized fatty acid composition.
6. A method according to paragraph 5, wherein the oxidized fatty acid composition is an oxidized tall oil fatty acid composition.
- 10 7. A method according to any of the preceding paragraphs, wherein the collector is an oxmal composition.
8. A method according to any of the preceding paragraphs, wherein the mineral is chosen from phosphate, barite, fluo-  
rite, feldspar, potash, fluorspar, magnesite, scheelite, cel-  
estite, anglesite, alunite, bauxite, gypsum, kainite, biotite,  
calcite, dolomite, albite, orthoclase, microcline, fluorspar,  
gypsum, anhydrite, columbite, tantalite, pyrochlore, apa-  
tite, cassiterite, wolframite, rutile, ilmenite, hematite, and  
kaolin.
9. A method according to paragraph 8, wherein the mineral is  
phosphate.
10. A method according to paragraph 8, wherein the mineral is  
potash.
11. A method according to any of the preceding paragraphs,  
wherein the method further comprises use of a frothing  
agent.
12. A method according to any of the preceding paragraphs,  
wherein the method further comprises use of a depressant.
13. A method of froth flotation comprising the use of a col-  
lector made by the process of:
  - providing a clean fatty acid composition; and
  - 35 oxidizing the clean fatty acid composition; to separate a  
mineral from gangue.
14. A method of froth flotation comprising the use of a col-  
lector made by the process of:
  - providing a fatty acid composition;
  - 40 maleating the fatty acid composition; and
  - oxidizing the fatty acid composition; to separate a min-  
eral from gangue.
15. A method of phosphate froth flotation comprising the use  
of a collector made by the process of:
  - providing a clean fatty acid composition; and
  - 45 oxidizing the clean fatty acid composition; to separate  
phosphate from gangue.
16. A method of phosphate froth flotation comprising the use  
of a collector made by the process of:
  - providing a fatty acid composition;
  - 50 maleating the fatty acid composition; and
  - oxidizing the fatty acid composition; to separate phos-  
phate from gangue.
17. A froth flotation process comprising collecting a mineral  
using an oxidized fatty acid composition, wherein the ox-  
idized fatty acid composition comprises less than 2.5% by  
55 weight of a plant-derived amine.
18. A froth flotation process comprising collecting a mineral  
using an oxidized fatty acid composition, wherein the ox-  
idized fatty acid composition comprises at least 65% by  
60 weight of an oxidized fatty acid.
19. A froth flotation process comprising collecting a mineral  
using an oxidized fatty acid composition, wherein the ox-  
idized fatty acid composition comprises less than 5% by  
65 weight of a tall oil pitch.
20. A froth flotation process comprising collecting a mineral  
using an oxidized fatty acid composition, wherein the ox-

- dized fatty acid composition comprises less than 20% by weight of a fuel oil or furnace oil.
21. A froth flotation process comprising collecting a mineral using an oxidized fatty acid composition, wherein the oxidized fatty acid composition has an acid value of at least about 80.
  22. A froth flotation process according to paragraph 21, wherein the oxidized fatty acid composition has an acid value of at least about 110.
  23. A froth flotation process according to paragraph 21, wherein the oxidized fatty acid composition has an acid value of between about 120 and about 150.
  24. A froth flotation process comprising collecting a mineral using an oxidized fatty acid composition and providing a yield of the mineral which is higher than a yield of the mineral provided by a fatty acid composition. 15
  25. A froth flotation process comprising collecting a mineral using an oxmal composition and providing a yield of the mineral which is higher than a yield of the mineral provided by a fatty acid composition.
  26. A froth flotation process comprising collecting a mineral using an oxidized fatty acid composition and providing a grade of the mineral which is higher than a grade of the mineral provided by a fatty acid composition. 20
  27. A froth flotation process comprising collecting a mineral using an oxmal composition and providing a grade of the mineral which is higher than a grade of the mineral provided by a fatty acid composition.
  28. A method of potash froth flotation, the method comprising floating potash using a collector comprising an oxidized fatty acid composition. 30
  29. A method of potash froth flotation, the method comprising floating potash using a collector comprising an oxmal composition.
  30. A method of separating a mineral from gangue, the method comprising providing an oxidized fatty acid composition to a solution of the mineral and gangue, thereby separating the mineral from the gangue.
  31. A method of separating a mineral from gangue, the method comprising providing an oxmal composition to a solution of the mineral and gangue, thereby separating the mineral from the gangue.
  32. A composition comprising a collector and a frothing agent, wherein the collector comprises one or more of an oxidized fatty acid composition, oxmal composition, and mixtures thereof. 45
  33. A composition comprising a collector and a depressant, wherein the collector comprises one or more of an oxidized fatty acid composition, oxmal composition, and mixtures thereof.
  34. A composition comprising two or more collectors, wherein at least one, but not all, of the collectors is an oxidized fatty acid.
  35. A kit comprising a collector and a frothing agent, wherein the collector comprises one or more of an oxidized fatty acid composition, oxmal composition, and mixtures thereof. 50
  36. A kit comprising a collector and a depressant, wherein the collector comprises one or more of an oxidized fatty acid composition, oxmal composition, and mixtures thereof.
  37. A kit according to one of paragraphs 35 and 36, wherein the kit further comprises instructions for floating a mineral.
  38. A kit according to one of paragraphs 35 and 36, wherein the kit further comprises a label that indicates that the contents are to be used in froth flotation of a mineral. 55

## EXAMPLES

## General Methods:

Acid value was determined using standard methods ASTM D 465-05 and AOCS Te 1 a-64. Standard test methods ASTM D 803-03 and AOCS Ja 10-87 (93) were used to measure Brookfield viscosity. Gardner-Holdt viscosity was determined using standard methods ASTM D1545-07 and AOCS Ja 11-87 (93). A hydrous acid number was obtained by titrating a sample of product dissolved in solvent (e.g., alcohol) using aqueous 0.5 N NaOH to a potentiometric endpoint (e.g., pH 13). All acid functionalities were titrated completely. The same ASTM test methodology as described above were used.

## Example 1

## Oxidized and Oxmal Compositions as Flotation Collectors in Phosphate Beneficiation

Phosphate ore can be beneficiated using the Crago Double Flotation process, in which the ore is first subjected to flotation using an anionic collector, and then the improved ore is subjected to a second "Reverse Flotation" using a cationic collector that floats clay and allows the improved phosphate ore to sink. This example addresses the first "Positive Flotation" using an anionic collector. The following reagents along with a proprietary commercial reagent were evaluated:

- (1) An oxidized TOFA composition;
- (2) XTOL® 100 (commercially available TOFA; used commercially as a component of a phosphate collector);
- (3) An oxidized and maleated TOFA composition;
- (4) A maleated TOFA composition;
- (5) A maleated and oxidized Crude Tall Oil composition; and
- (6) An oxidized and maleated 70:30 blend of TOFA and rosin.

Performance evaluation of the collectors in phosphate flotation was conducted under the following operating conditions:

40 The phosphate ore test sample was collected from central Florida. The phosphate sample was homogenized and split for analyses, storage and later usage. The acid insol (A.I.) content and  $P_2O_5$  grade of the phosphate was about 71.5% and 14.2%, respectively. The phosphate sample contained about 0.7% by weight particles larger than 16 mesh (1.18 mm). The 30-100 mesh particle size fraction accounted for more than 90% by weight of the same, while the 100-200 mesh fraction accounted for less than 1% by weight.

45 A Denver D-12 lab flotation machine equipped with a 2-liter tank was used for the phosphate flotation tests. Collector type, collector dosage and conditioning pH's were investigated in this study. The conditioning time and the impeller rotating speed were fixed at 2 minutes and 1500 rpm, respectively.

50 FIG. 1 shows the effects of collector dosage (ranging from 0.3 lb/ton to 0.9 lb/ton) on the percentage of phosphate flotation recovery was evaluated for each of the six collectors described above along with a typical commercial phosphate collector, labeled plant reagent. The curves indicate that flotation  $P_2O_5$  recovery increased significantly as the collector dosage increased from 0.3 lb/ton to 0.9 lb/ton. Collector (1), oxidized TOFA, showed a better percent recovery at all dosages than any of the other test samples including the typical commercial phosphate collector (plant reagent) and straight tall oil fatty acid (2), which has also been used as a commercial phosphate collector. Collector (1) achieved a maximum flotation  $P_2O_5$  recovery of 99.7% at a collector dosage of 0.9

39

lb/ton, while the commercial phosphate collector (plant reagent) when used at a dosage of 0.9 lb/ton achieved a maximum flotation recovery of 97.9%.

FIG. 2 illustrates the effects of collector dosage on percent  $P_2O_5$  recovery in the product for each of the experimental collectors including a typical commercial phosphate collector, labeled plant reagent. The curves indicate that percent  $P_2O_5$  in product reached a maximum for all reagents at 0.6 lb/ton. As with percent recovery, Collector (1), oxidized TOFA, yielded the highest percent  $P_2O_5$  in the product at all dosages compared to the other test collectors. Collector (1) achieved a concentrate of 20.4%  $P_2O_5$  at a collector dosage of 0.9 lb/ton. Comparatively, the commercial phosphate collector (plant reagent) when used at a dosage of 0.9 lb/ton achieved a concentrate grade of 19.8% P205.

FIG. 3 shows the effects of collector dosage on percent sols (acid solubles) in the product for each of the collectors. Percent sols in product is a measure of the amount of available phosphorus in the product. The curves indicate that percent  $P_2O_5$  in product reached a maximum for most reagents at 0.6 lb/ton. As with percent recovery and percent  $P_2O_5$  in product, Collector (1), oxidized TOFA, exhibited the highest percent sols in product at all dosages. Collector (3), an oxmal composition, showed strong performance as well especially compared to straight tall oil fatty acid (2). Collector (1) achieved a percent sols in product of 40.4% compared to 39.1% for the commercial phosphate collector (plant reagent) when used at a dosage of 0.9 lb/ton.

FIG. 4 shows the effects of collector type and dosage on phosphate separation efficiency, which is defined as the difference between  $P_2O_5$  recovery and A.I. recovery, i.e., separation efficiency=(%  $P_2O_5$  recovery-% A.I. rejection=100%). The curves indicate that separation efficiency increased as the collector dosage increased from 0.3 lb/ton to 0.6 lb/ton. The maximum separation efficiency with (1), plant reagent, and (3) was achieved at the collector dosages of about 0.6 lb/ton. At higher concentrations of collector the separation efficiency decreased due to a decrease in A.I. rejection. The separation efficiency with (1) was superior to all other collectors evaluated. As in the percent sols evaluation, Collector (3) outperformed Collector (2) XTOL® 100 in separation efficiency.

FIG. 5 illustrates the relationship between  $P_2O_5$  recovery and A.I. rejection for the seven collectors. The curves indicate that flotation  $P_2O_5$  recovery with Collector (1) was about 2% higher at a given A.I. rejection value compared to the plant reagent in the high  $P_2O_5$  recovery range. The fact that the Collector (1) curve was always above the plant reagent curve and, in fact, all other curves suggests that Collector (1) exhibited the highest separation efficiency.

In summary, the results shown in FIGS. 1-5 indicate that Collector (1) performed the best of the seven collectors for the

40

phosphate flotation under the conditions tested. In addition, Collector (3) exhibited superior phosphate flotation abilities compared to Collector (2) (XTOL® 100) in every test.

5

### Example 2

#### Preparation of Oxidized Tall Oil Fatty Acid

To a 2 liter flask fitted with a thermocouple, a fritted-glass sparge tube, a condenser, and a stirrer blade was added 1400.0 grams (4.87 moles) of tall oil fatty acid. The reaction flask was then heated to 165° C. Once the tall oil fatty acid reached a temperature of 155° C., an air sparge was applied to the reaction vessel at a rate of 4 liters/minute. Once the temperature reached 165° C., the reaction mixture was held at that temperature for 38 hours until the acid value was 120-140 mg KOH/g. The air sparge was then removed and the oxidized tall oil fatty acid was cooled to 60° C. and poured into a sample container. The physical properties for this product are as follows: Acid Value (mg KOH/g)=137.1; Brookfield Viscosity=3604 cPs (25° C., S #18, 100 rpm); Density (25° C.)=8.18 lbs/gal; Sp. Grav. (25° C.)=0.982.

25

### Example 3

#### Oxidation of Maleated Tall Oil Products

Two maleated tall oil products, XTOL® 690 and XTOL® 692, were oxidized using air at an elevated temperature. XTOL® 690 is a tall oil blend of tall oil fatty acid bottoms and a distilled tall oil, which blend has been maleated at a level of about 3.5%. XTOL® 692 is a blend of a tall oil rosin and tall oil fatty acid, which blend has been maleated at a level of about 12%.

Each of these tall oil blends was charged into a reactor which was fitted with an agitator, a thermocouple and a fritted glass sparge stone attached by a hose to an air supply. The tall oil blends were heated to 165° C. and the air turned on and adjusted to a flow rate of 4 L/hr through the sparge stone. The maleated tall oil reaction mixture was then heated to 177° C. and sampled frequently for acid value and viscosity (Gardner-Holdt) as the oxidation reactions proceeded, while holding the reaction mixture at a temperature of 177° C. The reaction mixture was held at a temperature of 177° C. for 10.5-16 hours as air was sparged. The reaction mixture was then cooled to 70-85° C. and discharged. The final physical properties of the maleated and oxidized tall oil product were determined as described above. The properties of the maleated and oxidized tall oil products were measured as shown in the following table with reference to typical properties of the starting materials:

|                                    | XTOL® 690 | Oxidized XTOL® 690 | XTOL® 692 | Oxidized XTOL® 692 |
|------------------------------------|-----------|--------------------|-----------|--------------------|
| Acid Value (mg KOH/g)              | 197.3     | 158.7              | 276.0     | 203.9              |
| Brookfield Viscosity (cPs; 25° C.) | 484.9     | 8496               | 1451      | 18010              |
| Density (Lbs./gal)                 | 8.00      | 8.38               | 8.41      | 8.59               |
| Sp. Gravity (25° C.)               | 0.961     | 1.006              | 1.010     | 1.031              |

-continued

| Description            | AcV<br>(cPs; 25° C.) | Visc  | GPC Results |      |      |             |      |      |
|------------------------|----------------------|-------|-------------|------|------|-------------|------|------|
|                        |                      |       | UV Detector |      |      | RI Detector |      |      |
|                        |                      |       | Mn          | Mw   | Mz   | Mn          | Mw   | Mz   |
| Oxidized XTOL ®<br>692 | 210.4                | 13560 | 654         | 1421 | 2884 | 519         | 844  | 1900 |
| Oxidized XTOL ®<br>690 | 158.7                | 8970  | 800         | 3410 | 9378 | 618         | 1959 | 7330 |

## Example 4

## Maleation of Oxidized Tall Oil

An oxidized and maleated tall oil composition was produced through the maleation of a commercially available oxidized tall oil product. The oxidized tall oil product, XTOL® MTO, which is an oxidized, high acid value crude tall oil, available commercially from Georgia Pacific was used as the starting material. This oxidized crude tall oil was treated with maleic anhydride.

XTOL® MTO (95 wt %) was charged to a sealed reactor fitted with an agitator, a thermocouple and a condenser. The reactor was heated to 180° C. At 180° C. maleic anhydride (5 wt %) was added slowly to the reactor. The reaction mixture was then heated to 200° C. for approximately 3-6 hours or until all of the maleic anhydride had reacted. The reaction mixture was then cooled to 70-80° C. and discharged. The final physical properties were determined as described above. The properties of the oxidized and maleated tall oil product were measured as shown in the following table with reference to typical properties of the starting materials:

|                                    | XTOL ®<br>MTO | Maleated XTOL ® MTO<br>(Oxidized tall oil) |
|------------------------------------|---------------|--------------------------------------------|
| Acid Value                         | 143.0         | 163.8                                      |
| Density (25° C.; Lbs./gal)         | 8.25          | 8.52                                       |
| Sp. Gravity (25° C.)               | 0.99          | 1.023                                      |
| Brookfield Viscosity (cPs; 25° C.) | 4870          | 22580                                      |

## Example 5

## Maleation of Crude Tall Oil Followed by Oxidation

A process similar to the one described in Example 1 was used, whereby a crude tall oil mixture was maleated followed by oxidation. In this specific example, the composition was maleated to a level of about 5% and then oxidized.

A crude tall oil (95 wt. %) was charged to a sealed reactor fitted with an agitator, a thermocouple, and a condenser. The reaction mixture was heated to 180° C. At 180° C., maleic anhydride (5 wt. %) was added slowly to the reactor. The reaction mixture was then heated to 200° C. for approximately 3-6 hours or until all of the maleic anhydride had reacted. Once all of the maleic anhydride had reacted, the reaction mixture was then cooled to 180° C. and air was introduced to the reaction mixture using a fritted glass sparge stone attached by a hose to an air supply. The air was turned on and adjusted to a flow rate of 4 L/hr through the sparge stone. Oxidation of the maleated crude tall oil with air was carried out for 12-16 hours. The reaction mixture was then cooled to 70-85° C. and discharged. The final physical properties were determined. The properties of the maleated and oxidized tall oil product were measured as shown in the

following table with reference to typical properties of the starting materials:

|                                    | Crude Tall Oil | Maleated-Oxidized<br>Crude tall oil |
|------------------------------------|----------------|-------------------------------------|
| Acid Value                         | 161.6          | 169.5                               |
| Density (25° C.; Lbs./gal)         | 8.088          | 8.54                                |
| Specific Gravity (25° C.)          | 0.9706         | 1.027                               |
| Brookfield Viscosity (cPs; 25° C.) | 695.0          | 33800                               |

## Example 6

## Oxidation of Maleated Tall Oil Fatty Acid

In this example, a maleated tall oil fatty acid (TOFA) was oxidized using air at an elevated temperature.

TOFA was charged to a sealed reactor and the contents of the reactor were heated to 70° C. Once a temperature of 70° C. was achieved, maleic anhydride in an amount of about 25% by weight of the overall reaction was added to the vessel. The reactor mixture was then heated to 220° C. in several stages. From the starting temperature of 70° C., the temperature was increased in small increments until 220° C. was achieved. After each temperature adjustment and the desired set point was reached, the material was maintained at the set point temperature for a five minute hold period. The first stage of heating was from 70° C. to 130° C.; the second stage of heating was from 130° C. to 160° C.; the third stage of heating was from 160° C. to 185° C.; the fourth stage of heating was from 185° C. to 205° C.; and the fifth and final stage of heating was from 205° C. to 220° C. The reaction mixture then was held at 220° C. until a Gardner-Holdt viscosity of about Z-2 was reached. This holding period typically required about 5 hours depending on the batch size. The reaction mixture was cooled to a discharge temperature and the physical properties of the maleated product were measured as described above. Typically, the maleated product exhibited an acid number (hydrous) equal to 300-320 mg KOH/g, a specific gravity of 1.04 and a Brookfield Viscosity (at 25° C.) equal to 2700-3400 cps.

To produce a maleated and oxidized fatty acid composition, the maleated tall oil fatty acid was then charged to a reactor which was fitted with an agitator, a thermocouple, and a fritted glass sparge stone attached by a hose to an air supply. The maleated tall oil fatty acid was heated to 165° C. and the air was turned on and adjusted to a flow rate of 4 L/hr through the sparge stone. The reaction mixture was then heated to 177° C. and sampled frequently for acid value and viscosity (Gardner-Holdt) while holding the reaction mixture at 177° C. The reaction mixture was held at 177° C. for 10.5-16 hours as air was sparged. The reaction mixture was then cooled to 70-85° C. and discharged. The final physical properties of the maleated and oxidized TOFA were then determined as described above. The properties of the maleated and oxidized TOFA were measured as:

| Oxidized Maleated<br>Tall Oil Fatty Acid |                     |       |             |      |      |             |     |      |
|------------------------------------------|---------------------|-------|-------------|------|------|-------------|-----|------|
| GPC Results                              |                     |       |             |      |      |             |     |      |
| Description                              | AcV<br>(cPs; 25 C.) | Visc  | UV Detector |      |      | RI Detector |     |      |
|                                          |                     |       | Mn          | Mw   | Mz   | Mn          | Mw  | Mz   |
| Oxidized Maleated<br>TOFA                | 258.5               | 13560 | 830         | 1503 | 2678 | 654         | 908 | 1603 |
| Oxidized Maleated<br>TOFA                | 247.3               | 19328 | 841         | 1535 | 2759 | 644         | 879 | 1548 |

## Example 7

## Oxidation of Maleated Arachidonic Acid (ARA)

In this example, a maleated arachidonic acid (ARA) is oxidized using air at an elevated temperature. Arachidonic acid is produced by the saponification of natural fish oils and is particularly prevalent in sardine oil.

ARA is charged to a sealed reactor and the contents of the reactor are heated to 70° C. Once a temperature of 70° C. is achieved, maleic anhydride in an amount of about 40% by weight of the total reaction is added to the vessel. The reactor mixture is then heated to 220° C. in several stages. From the starting temperature of 70° C., the temperature is increased in small increments until 220° C. is achieved. After each temperature adjustment and the desired set point is reached, the material is maintained at the set point temperature for a five minute hold period. The first stage of heating is from 70° C. to 130° C.; the second stage of heating is from 130° C. to 160° C.; the third stage of heating is from 160° C. to 185° C.; the fourth stage of heating is from 185° C. to 205° C.; and the fifth and final stage of heating is from 205° C. to 220° C. The reaction mixture then is held at 220° C. until a Gardner-Holdt viscosity of about Z-2 is reached. This holding period varies depending on the batch size. The reaction mixture is cooled to a discharge temperature and the physical properties of the maleated product are measured as described in previous examples.

To produce a maleated and oxidized ARA composition, the maleated ARA is then charged to a reactor which is fitted with an agitator, a thermocouple, and a fritted glass sparge stone attached by a hose to an air supply. The maleated ARA is heated to 165° C. and the air is turned on and adjusted to a flow rate of 4 L/hr through the sparge stone. The reaction mixture is then heated to 177° C. and sampled frequently for the acid value and viscosity (Gardner-Holdt) that is appropriate for the specific application while holding the reaction mixture at 177° C. The reaction mixture is held at 177° C. for the length of time necessary to achieve the desired acid value and viscosity as air is sparged. The reaction mixture is then cooled to 70-85° C. and discharged.

A non-limiting example of a compound produced by the above procedure is:



## Example 8

## Production of a Na Salt of an Oxidized Tall Oil Fatty Acid

A 250-mL stainless steel beaker was placed in a sand bath which was capable of heating. To the 250-mL stainless steel beaker was added 100.49 g (0.245 moles) of an oxidized tall oil fatty acid. A mechanical stirrer and a thermocouple were placed in the beaker. The oxidized tall oil fatty acid was slowly heated to 60° C. while stirring vigorously. Once the temperature in the beaker reached 60° C., 20.34 g (0.249 moles) of 48.9% NaOH solution was added dropwise over a twenty minute period. During the NaOH addition, an exotherm was experienced in the reaction mixture which increased the temperature to 80° C. Once the addition of the NaOH was complete, 106.14 grams of deionized water was added slowly with vigorous stirring to dilute the reaction mixture to 48.60% solids. The final pH of the solution was 9.43.

45

Example 9

## Production of a Na Salt of an Oxmal Composition

A 250-mL stainless steel beaker was placed in a sand bath which was capable of heating. To the 250-mL stainless steel beaker was added 100.14 g (0.353 moles) of an oxmal composition. A mechanical stirrer and a thermocouple were placed in the beaker. The oxmal composition was slowly heated to 60° C. while stirring vigorously. Once the temperature in the beaker reached 60° C., 28.87 g (0.353 moles) of 48.9% NaOH solution was added, dropwise, over a twenty minute period. During the NaOH addition, an exotherm was experienced in the reaction mixture which increased the temperature to 90° C. Once the addition of the NaOH was complete, 99.68 grams of deionized water was added slowly with vigorous stirring to dilute the reaction mixture to 49.96% solids. The final pH of the solution was 9.00.

A number of embodiments have been described. Nevertheless, it will be understood that various modifications may be made without departing from the spirit and scope of the disclosure. Accordingly, other embodiments are within the scope of the following claims.

What is claimed is:

1. A method of froth flotation for the beneficiation of an ore, the method comprising:
  - contacting a slurry comprising an ore with a collector, wherein the collector comprises one or more compounds or salts thereof having at least two  $C_{10}$ - $C_{24}$  structures crosslinked by an ether linkage; and recovering a beneficiated ore.
  2. A method according to claim 1, wherein the at least two  $C_{10}$ - $C_{24}$  structures comprise clean fatty acids, tall oil fatty acids, or mixtures thereof.
  3. A method according to claim 1, wherein the at least two  $C_{10}$ - $C_{24}$  structures comprise tall oil fatty acids.
  4. A method according to claim 1, wherein the collector is an anionic collector.
  5. A method according to claim 4, wherein the anionic collector has a counter cation chosen from  $Li^+$ ,  $Na^+$ ,  $K^+$ ,  $NH_4^+$ , alkyl ammonium ions, and imidazoline cations.
  6. A method according to claim 1, wherein the at least two  $C_{10}$ - $C_{24}$  structures comprise clean fatty acids, wherein the clean fatty acids does not contain one or more of tall oil pitch, an amine, or sarcosine.
  7. A method according to claim 1, wherein a grade of the beneficiated ore is greater than a grade of a beneficiated ore recovered with a comparative collector comprising one or more compounds or salts thereof having at least two  $C_{10}$ - $C_{24}$  structures not crosslinked by an ether linkage.
  8. A method according to claim 1, wherein at least one of the  $C_{10}$ - $C_{24}$  structures is substituted by at least one  $\alpha,\beta$  unsaturated carboxylic acid or anhydride.
  9. A method according to claim 1, wherein the ore is chosen from phosphate, barite, fluorite, feldspar, potash, fluorspar, magnesite, scheelite, celestite, anglesite, alunite, bauxite, gypsum, kainite, biotite, calcite, dolomite, albite, orthoclase, microcline, fluorspar, gypsum, anhydrite, columbite, tanta-

46

lite, pyrochlore, apatite, cassiterite, wolframite, rutile, ilmenite, hematite, and kaolin.

10. A method according to claim 9, wherein the beneficiated ore is phosphate.
11. A method according to claim 9, wherein the beneficiated ore is potash.
12. A method according to claim 1, wherein the method further comprises use of a frothing agent.
13. A method according to claim 1, wherein the method further comprises use of a depressant.
14. A method according to claim 1, wherein the collector has at least one characteristic chosen from: the collector comprises less than 2.5% by weight of a plant-derived amine, the collector comprises at least 65% by weight of a fatty acid, the collector, comprises less than 5% by weight of a tall oil pitch, the collector, comprises less than 20% by weight of a fuel oil or furnace oil, and the collector has an acid value of at least about 80.
15. A method according to claim 3, wherein the collector has an acid value of at least about 110.
16. A method according to claim 3, wherein the collector has an acid value ranging from about 120 to about 150.
17. A method according to claim 1, wherein a yield of the beneficiated ore is greater than a yield of a comparative beneficiated ore recovered with a comparative collector comprising one or more compounds or salts thereof having at least two  $C_{10}$ - $C_{24}$  structures not crosslinked by an ether linkage.
18. A method according to claim 3, wherein the collector has less than 20% by weight of a fuel oil.
19. A method according to claim 8, further comprising collecting the mineral and providing one or more of: a yield of the mineral which is higher than a yield of the mineral provided by a fatty acid composition, and a grade of the mineral which is higher than a grade of the mineral provided by a fatty acid composition.
20. A method according to claim 8, wherein the collector has an acid value of at least about 110.
21. A method of froth flotation comprising:
  - contacting an aqueous slurry comprising a mineral and gangue with a first collector, wherein the first collector comprises one or more compounds or salts thereof having at least two  $C_{10}$ - $C_{24}$  structures crosslinked by an ether linkage made by sparging air through a reaction mixture composed of tall oil fatty acids at a temperature of at least 150° C.; and
  - separating the mineral from the gangue.
22. A method according to claim 21, wherein the reaction mixture is heated to a temperature of about 160° C. to about 170° C.
23. A method according to claim 21, wherein the mineral is phosphate.
24. A method according to claim 21, wherein the at least two  $C_{10}$ - $C_{24}$  structures crosslinked by an ether linkage are reacted with maleic anhydride or maleic acid such that at least one of the  $C_{10}$ - $C_{24}$  structures is substituted by at least one  $\alpha,\beta$  unsaturated carboxylic acid or anhydride.

\* \* \* \* \*